# EUROPEAN PATENT APPLICATION

(11) **EP 3 241 979 A1**
(43) Date of publication of application: **08.11.2017**
(21) Application number: 17169004.3
(22) Date of filing: 02.05.2017
(51) Int. Cl.: E21B 23/00

(54) **DEGRADABLE CARBIDE GRIP**

(30) Priority: 02.05.2016 US 201662330794 P; 28.04.2017 US 201715499988
(71) Applicant: Services Pétroliers Schlumberger, 75007 Paris (FR); Schlumberger Technology B.V., 2514 JG The Hague (NL)
(72) Inventor: INDRANIL, Roy, Rosharon, TX Texas 77583 (US); JACOB, Gregoire, Rosharon, TX Texas 77583 (US); BAILONI, Sergio, Trento Trento (IT)
(74) Representative: Schlumberger Cambridge Research Limited

(57) **Abstract**

An apparatus can include a degradable matrix that is degradable in an aqueous environment; and non-degradable particles disposed at least in part within the matrix where the non-degradable particles are not degradable in the aqueous environment where the non-degradable particles can include tungsten carbide.

## Description

### BACKGROUND

Various types of materials are used in equipment, operations, etc. for exploration, development and production of resources from geologic environments. For example, equipment may be used in one or more of a sensing operation, a drilling operation, a cementing operation, a fracturing operation, a production operation, etc.

### SUMMARY

An apparatus can include a degradable matrix that is degradable in an aqueous environment; and non-degradable particles disposed at least in part within the matrix where the non-degradable particles are not degradable in the aqueous environment where the non-degradable particles can include tungsten carbide. A method can include
pressing a blend of materials where the materials include a non-degradable material that is not degradable in an aqueous environment and an aqueous degradable alloy material; and forming a grip from the pressed blend of materials. An assembly can include a plurality of components where at least one of the components includes a grip that includes a degradable matrix that is degradable in an aqueous environment and non-degradable particles disposed at least in part within the matrix where the non-degradable particles are not degradable in the aqueous environment and where the non-degradable particles include tungsten carbide. Various other apparatuses, systems, methods, etc., are also disclosed.

This summary is provided to introduce a selection of concepts that are further described below in the detailed description. This summary is not intended to identify key or essential features of the claimed subject matter, nor is it intended to be used as an aid in limiting the scope of the claimed subject matter.

### BRIEF DESCRIPTION OF THE DRAWINGS

Features and advantages of the described implementations can be more readily understood by reference to the following description taken in conjunction with the accompanying drawings.
Figs. 1 and 2 illustrate an example of a method and examples of equipment for fracturing a geologic environment;
Fig. 3 illustrates an example of equipment in various example operational states;
Fig. 4 illustrates an example of a method;
Fig. 5 illustrates an example of a method;
Fig. 6 illustrates an example of a metal matrix composite material;
Fig. 7 illustrates an example of a method;
Fig. 8 illustrates micrographs of an example of a degradable material;
Fig. 9 illustrates an example of a component;
Fig. 10 illustrates an example of a component;
Fig. 11 illustrates an image of an example of an interface of an example of a component;
Fig. 12 illustrates an example of an arrangement of components;
Fig. 13 illustrates an example of an assembly and an example of a grip;
Fig. 14 illustrates an example of an assembly;
Fig. 15 illustrates an example of an assembly;
Fig. 16 illustrates an example of a disc and examples of grips formed from the disc;
Fig. 17 illustrates an example of a press;
Fig. 18 illustrates an example of a method;
Fig. 19 illustrates examples of grips;
Fig. 20 illustrates examples of grips;
Fig. 21 illustrates an example of an assembly that includes a grip;
Fig. 22 illustrates an example of a system;
Fig. 23 illustrates an example of a micrograph of an example of particles;
Fig. 24 illustrates an example of a micrograph of an example of a particle;
Fig. 25 illustrates an example of a micrograph of an example of a particle;
Fig. 26 illustrates an example of a plot of a component parameter versus degradation time, an example of an assembly and examples of components;
Fig. 27 illustrates examples of equipment;
Fig. 28 illustrates an example of a life cycle; and
Fig. 29 illustrates example components of a system and a networked system.

### DETAILED DESCRIPTION

The following description includes the best mode presently contemplated for practicing the described implementations. This description is not to be taken in a limiting sense, but rather is made merely for the purpose of describing the general principles of the implementations. The scope of the described implementations should be ascertained with reference to the issued claims.

As an example, a material or materials may be processed to form processed material. In such an example, the processed material may be compressed, machined, formed, etc. to produce a part or parts. As an example, a part may be a component or a portion of a component. A part may be included in equipment, which may be suitable for use in an environment such as, for example, a downhole environment. As an example, equipment may be drilling equipment, cementing equipment, fracturing equipment, sampling equipment, or other type of equipment. As an example, equipment may be borehole equipment. As an example, a tool may be a borehole tool, for example, suitable to perform a function or functions in a downhole environment in a borehole.

As to cementing equipment, such equipment may be used in one or more downhole cementing operations. As an example, cement may be placed adjacent to a liner. As an example, a liner may be a string of casing in which the top does not extend to the surface but instead is suspended from inside another casing string. As an example, a liner hanger may be used to attach or hang one or more liners from an internal wall of another casing string.

As an example, a method may include operating one or more components of a liner hanger system. As an example, a lower completion may be a portion of a well that is at least in part in a production zone or an injection zone. As an example, a liner hanger system may be implemented to perform one or more operations associated with a lower completion, for example, including setting one or more components of a lower completion, etc. As an example, a liner hanger system may anchor one or more components of a lower completion to a production casing string.

As an example, equipment may include one or more plugs, one or more seats that can receive a respective plug, etc. In such an example, it may be desirable that a plug and/or a seat have properties suited for one or more operation or operations. Properties may include mechanical properties and may include one or more other types of properties (e.g., chemical, electrical, etc.). As an example, it may be desirable that a plug and/or a seat degrade. For example, a plug and/or a seat may be manufactured with properties such that the plug and/or the seat degrade when exposed to one or more conditions. In such an example, where the plug acts to block a passage, upon degradation, the passage may become unblocked. As an example, a component (e.g., a plug, a seat, a grip, etc.) may degrade in a manner that facilitates one or more operations. As an example, a component or a portion of a component may degrade in stages. For example, consider a plug that degrades from a first size to a second smaller size. In such an example, the second smaller size may allow the plug to move (e.g., from a first seat to a second seat, etc.). As an example, a plug tool may be a degradable tool. As an example, a plug tool may be degradable in part. For example, consider a plug tool with a degradable seat or degradable seats. In such an example, a plug may be seated in a degradable seat that upon degradation of the seat, the plug may pass through the seat (e.g., become unplugged with respect to that seat). As an example, a system can include a plug tool that is degradable at least in part and can also include one or more degradable plugs (e.g., balls, cylinders, etc.).

As an example, at least a portion of a borehole tool may be broken via interaction with a tool where at least some of resulting pieces are degradable. For example, a tool may apply force (e.g., drilling force or other force) to a plug, a plug tool, a grip, etc. such that the applied forces cause breaking into pieces of at least a portion of the plug, at least a portion of the plug tool, at least a portion of the grip, etc. In such an example, the pieces may be relatively large and degrade to relatively small pieces (e.g., which may pass through one or more openings, etc.).

As an example, equipment may include one or more elastomeric components. An elastomer can be defined as being a polymeric material characterized by at least some amount of viscoelasticity (e.g., viscosity and elasticity). As an example, an elastomer can have a relatively low Young's modulus and, for example, a relatively high failure strain compared to various other materials. An example of an elastomer is rubber, which can include vulcanizates.

In an elastomer, monomers can be linked to form a backbone, chains, a network, etc. As an example, an elastomer can include one or more of carbon, hydrogen, oxygen and silicon. Elastomers may be characterized as being amorphous polymeric materials that exist above their glass transition temperature, for example, such that considerable segmental motion is possible. At ambient temperatures, rubbers tend to be relatively soft (e.g., consider a Young's modulus "E" of about 3 MPa) and deformable. Elastomers may be used, for example, as seals, adhesives, molded flexible parts, etc. As an example, an elastomer may be a damping element, an insulating element, a seal element, etc.

As an example, a seal element may include an elastomer, optionally in addition to one or more other materials. As an example, a component can include a material that is relatively rigid and a material that is elastomeric. For example, consider a component where an elastomer covers at least a portion of a metal or metal alloy structure. In such an example, the elastomer may impart surface properties that can assist with an operation, a function, etc., of a component.

As an example, particles may be added to a polymeric material where at least a portion of the particles are degradable. For example, degradable particles may be added to polymeric material such that a composite polymeric material is degradable, for example, upon exposure to water. As an example, a composite polymeric material may include carbon particles (e.g., carbon black, carbon nanotubes, graphene, etc.) and degradable material particles. As to degradable particles, these can include aluminum as an alloying element in combination with one or more other elements.

As an example, a grip or grips may act to position one or more components. As an example, a grip or grips may act to locate one or more components in a borehole. Such a grip or grips may act to locate a component in a relative position and/or orientation with respect to another component. As an example, a component may be fixed in its position, for example, due to cementing or other binding to earth. As an example, a component may be movable in a borehole or components may be movable in a borehole. As an example, a grip or grips may act to locate one movable component with respect to another movable component. As an example, during an operation, a movable component may be anchored via a grip or grips. As an example, where a grip and/or a component is degradable, position of the grip and/orthe component may change upon degradation of the grip and/or the component.

As an example, a grip or grips may act to anchor a component, an assembly, etc. For example, a grip may contact a surface of a pipe and contact a surface of a component to act to anchor the component with respect to the pipe. As an example, a pipe may be a casing such as, for example, a low alloy steel (LAS) casing.

Alloy steel is steel that is alloyed with a variety of elements in total amounts between about 1.0 percent and about 50 percent by weight, for example, to enhance mechanical properties. Alloy steels may be classified as being low alloy steel or high alloy steel, which may defined using a weight percent of alloy of about 4 percent to about 8 percent. Alloy steel alloyants may include, for example, one or more of manganese, nickel, chromium, molybdenum, vanadium, silicon, boron, aluminum, cobalt, copper, cerium, niobium, titanium, tungsten, tin, zinc, lead, and zirconium.

As an example, a high-strength low alloy steel (HSLAS) may have a yield strength greater than about 250 MPa or about 36 ksi. HSLAS can be suitable for use in oil and/or gas pipelines. As an example, HSLAS AISI 4130 (e.g., or modification thereof) may be utilized for pipe, tubing, liner, casing, etc. in a well. Composition of AISI 4130 can be, for example, within ranges as follows by weight percentage: C 0.28 - 0.33; Cr 0.8 - 1.1; Fe 97.3 - 98.2; Mn 0.4 - 0.6; Mo 0.15 - 0.25; P Max 0.035; S Max 0.04; Si 0.15 - 0.35. As an example, AISI 4130 may have a Vickers hardness of about 207 (e.g., Brinell hardness of about 197) and a yield strength of about 435 MPa (e.g., about 63 ksi). As an example, 316L stainless steel can exhibit a Vickers hardness of about 140; whereas diamond can exhibit a Vickers hardness of about 10,000. As an example of another hard material, consider martensite with a Vickers hardness of about 1,000; noting that hard crystalline or polycrystalline materials may fracture rather than "indent" (e.g., exhibit an indentation fracture hardness).

As an example, a grip can have a hardness that exceeds the hardness of another component. For example, a grip may have a hardness that exceeds a hardness of a LAS. As an example, hardness may be determined using a Vickers hardness test where an indenter is pressed against a test material. As an example, an indenter can be a pyramidal diamond that is loaded for a period of time (e.g., 30 kgf for 10 seconds).

As an example, a grip can be degradable where a degradable material forms a matrix that can include a hard material. For example, consider a composite material that includes a degradable alloy matrix and polycrystalline diamonds disposed within the matrix. As another example, consider a material that includes a degradable alloy matrix and one or more ceramic materials disposed within the matrix. As an example, a material can include a degradable material and a non-degradable material; where degradable means degradable in an aqueous environment, which may be found, for example, in a well. As an example, a degradable material may be referred to as a water reactive material.

As an example, a water reactive or degradable anchoring device can be an engineered part made from a metal matrix composite (MMC) or alloy that is capable of biting or anchoring into a low alloy steel casing, that exhibits adequate hardness, and that is water reactive. In such an example, the anchoring device may include degradable material that degrades at a rate that is sufficiently slow enough to complete one or more operations before losing its anchoring capability. For example, consider an anchoring device that can anchor to casing and that can be utilized for a stimulation operation before dislodging from the casing.

As mentioned, equipment may include fracturing equipment where such equipment may be employed to generate one or more fractures in a geologic environment. As an example, a method to generate fractures can include a delivery block for delivering fluid to a subterranean environment, a monitor block for monitoring fluid pressure and a generation block for generating fractures via fluid pressure. As an example, the generation block may include activating one or more fractures. As an example, the generation block may include generating and activating fractures. As an example, activation may occur with respect to a pre-existing feature such as a fault or a fracture. As an example, a pre-existing fracture network may be at least in part activated via a method that includes applying fluid pressure in a subterranean environment. The foregoing method may be referred to as a treatment method or a "treatment". Such a method may include pumping an engineered fluid (e.g., a treatment fluid) at high pressure and rate into a reservoir via one or more bores, for example, to one or more intervals to be treated, which may cause a fracture or fractures to open (e.g., new, pre-existing, etc.).

As an example, a fracture may be defined as including "wings" that extend outwardly from a bore. Such wings may extend away from a bore in opposing directions, for example, according in part to natural stresses within a formation. As an example, proppant may be mixed with a treatment fluid to keep a fracture (or fractures) open when a treatment is complete. Hydraulic fracturing may create high-conductivity communication with an area of a formation and, for example, may bypass damage that may exist in a near-wellbore area. As an example, stimulation treatment may occur in stages. For example, after completing a first stage, data may be acquired and analyzed for planning and/or performance of a subsequent stage.

Size and orientation of a fracture, and the magnitude of the pressure to create it, may be dictated at least in part by a formation's in situ stress field. As an example, a stress field may be defined by three principal compressive stresses, which are oriented perpendicular to each other. The magnitudes and orientations of these three principal stresses may be determined by the tectonic regime in the region and by depth, pore pressure and rock properties, which determine how stress is transmitted and distributed among formations.

Where fluid pressure is monitored, a sudden drop in pressure can indicate fracture initiation of a stimulation treatment, as fluid flows into the fractured formation. As an example, to break rock in a target interval, fracture initiation pressure exceeds a sum of the minimum principal stress plus the tensile strength of the rock. To determine fracture closure pressure, a process may allow pressure to subside until it indicates that a fracture has closed. A fracture reopening pressure may be determined by pressurizing a zone until a leveling of pressure indicates the fracture has reopened. The closure and reopening pressures tend to be controlled by the minimum principal compressive stress (e.g., where induced downhole pressures exceed minimum principal stress to extend fracture length).

After performing fracture initiation, a zone may be pressurized for furthering stimulation treatment. As an example, a zone may be pressurized to a fracture propagation pressure, which is greater than a fracture closure pressure. The difference may be referred to as the net pressure, which represents a sum of frictional pressure drop and fracture-tip resistance to propagation (e.g., further propagation).

As an example, a method may include seismic monitoring during a treatment operation (e.g., to monitor fracture initiation, growth, etc.). For example, as fracturing fluid forces rock to crack and fractures to grow, small fragments of rock break, causing tiny seismic emissions, called microseisms. Equipment may be positioned in a field, in a bore, etc. to sense such emissions and to process acquired data, for example, to locate microseisms in the subsurface (e.g., to locate hypocenters). Information as to direction of fracture growth may allow for actions that can "steer" a fracture into a desired zone(s) or, for example, to halt a treatment before a fracture grows out of an intended zone. Seismic information (e.g., information associated with microseisms) may be used to plan one or more stages of fracturing operations (e.g., location, pressure, etc.).

Figs. 1 and 2 show an example of a method 100 that includes generating fractures. As shown, the method 100 can include various operational blocks such as one or more of the blocks 101, 102, 103, 104, 105 and 106. The block 101 may be a drilling block that includes drilling into a formation 110 that includes layers 112, 114 and 116 to form a bore 130 with a kickoff 132 to a portion defined by a heel 134 and a toe 136, for example, within the layer 114.

As illustrated with respect to the block 102, the bore 130 may be at least partially cased with casing 140 into which a string or line 150 may be introduced that carries a perforator 160. As shown, the perforator 160 can include a distal end 162 and charge positions 165 associated with activatable charges that can perforate the casing 140 and form channels 115-1 in the layer 114. Next, per the block 103, fluid may be introduced into the bore 130 between the heel 134 and the toe 136 where the fluid passes through the perforations in the casing 140 and into the channels 115-1. Where such fluid is under pressure, the pressure may be sufficient to fracture the layer 114, for example, to form fractures 117-1. In the block 103, the fractures 117-1 may be first stage fractures, for example, of a multistage fracturing operation.

Per the block 104, additional operations are performed for further fracturing of the layer 114. For example, a plug 170 may be introduced into the bore 130 between the heel 134 and the toe 136 and positioned, for example, in a region between first stage perforations of the casing 140 and the heel 134. Per the block 105, the perforator 160 may be activated to form additional perforations in the casing 140 (e.g., second stage perforations) as well as channels 115-2 in the layer 114 (e.g., second stage channels). Per the block 106, fluid may be introduced while the plug 170 is disposed in the bore 130, for example, to isolate a portion of the bore 130 such that fluid pressure may build to a level sufficient to form fractures 117-2 in the layer 114 (e.g., second stage fractures).

In a method such as the method 100 of Figs. 1 and 2, it may be desirable that a plug (e.g., the plug 170) includes properties suited to one or more operations. Properties of a plug may include mechanical properties (e.g., sufficient strength to withstand pressure associated with fracture generation, etc.) and may include one or more other types of properties (e.g., chemical, electrical, etc.). As an example, it may be desirable that a plug degrades, that a plug seat degrades, that at least a portion of a borehole tool degrades, etc. For example, a plug may be manufactured with properties such that the plug withstands, for a period of time, conditions associated with an operation and then degrades (e.g., when exposed to one or more conditions). In such an example, where the plug acts to block a passage for an operation, upon degradation, the passage may become unblocked, which may allow for one or more subsequent operations. As an example, the method 100 may employ one or more grips, which may optionally include one or more degradable grips.

As an example, a component may be degradable (e.g., a grip or other type of component) upon contact with a fluid such as an aqueous ionic fluid (e.g., saline fluid, etc.). As an example, a component may be degradable upon contact with well fluid that includes water (e.g., consider well fluid that includes oil and water, etc.). As an example, a component may be degradable upon contact with a fracturing fluid (e.g., a hydraulic fracturing fluid). Fig. 15 shows an example plot 1500 of degradation time versus a component dimension for various temperatures where a component is in contact with a fluid that is at least in part aqueous (e.g., include water as a medium, a solvent, a phase, etc.).

Fig. 3 shows an example of equipment in various states 301, 302 and 303. As shown, the equipment can include a casing 340 that include various components 341, 342, 343 and 345. For example, the component 342 may define a bore 346 and the component 345 may define a bore 348 where the component 343 includes features (e.g., reduced diameter, conical shape, receptacle, etc.) that can catch a ring component 370 that is operatively coupled to a plug component 360 where the ring component 370 and the plug component 360 may position and seat a plug 350 in the casing 340. As an example, a seal may be formed by the plug 350 with respect to the plug component 360 and/or the ring component 370 and, for example, a seal may be formed by the ring component 370 with respect to the component 343. In such an approach, the seals may be formed in part via fluid pressure in a manner where increased pressure acts to increase seal integrity (e.g., reduce clearances that may be subject to leakage). As an example, the ring component 370 may be an upper component (e.g., a proximal component) of a plug seat and the plug component 360 may be a lower component (e.g., a distal component) of the plug seat.

As shown in the state 301, the plug 350 may be seated such that the bore 346 (e.g., of a first zone) is separated (e.g., isolated) from the bore 348 (e.g., of a second zone) such that fluid pressure in the bore 346 (see, e.g., P₂) may be increased to a level beyond fluid pressure in the bore 348 (see, e.g., P₁). Where the plug 350 and the plug component 360 are degradable, for example, upon contact with fluid that may pressurize the bore 348, degradation of the plug 350 and the plug component 360 may transition the equipment from the state 301 to the state 302. As shown in the state 302, fluid may pass from the bore 346 to the bore 348, for example, via an opening of the ring component 370. Where the ring component 370 is degradable, for example, upon contact with fluid in the bore 346, degradation of the ring component 370 may transition the equipment from the state 302 to the state 303. In the state 303, the casing 340 may be the remaining equipment of the state 301 (e.g., the plug 350, the plug component 360 and the ring component 370 are at least in part degraded).

As an example, the plug 350, the plug component 360 and the ring component 370 may be components of a dissolvable plug and perforation system that may be used to isolate zones during stimulation (see, e.g., the method 100 of Figs. 1 and 2). Such equipment may be implemented in, for example, cemented, uncemented, vertical, deviated, or horizontal bores (e.g., in shale, sandstone, dolomite, etc.).

As an example, the plug component 360 and the ring component 370 may be conveyed in a bore via a pump down operation (e.g., which may move the components 360 and 370 along a bore axis direction). As an example, a component or components may include adjustable features, for example, that allow a change in diameter to facilitate seating in a receptacle disposed in a bore. For example, a tool may interact with a component or components to cause a change in diameter or diameters (e.g., a change in form of one or more components). In the changed state, the component or components may catch and seat in a receptacle disposed in a bore (e.g., seat in a shoulder of a receptacle component).

As an example, the plug component 360 and the ring component 370 may be seated in a receptacle by a tool that may include one or more perforators. Once seated, the tool may be repositioned to perforate casing and form channels (e.g., in a layer or layers of rock). As an example, repositioning may occur multiple times, for example, to form multiple sets of perforations and multiple sets of channels. As an example, after perforating and channel formation, the plug 350 may be pumped down to contact the plug component 360 and/or the ring component 370, for example, to form a seal that can isolate one zone from another zone (e.g., one interval from another interval). Fluid pressure may be increased in an isolated zone as defined by the plug 350, the plug component 360 and the ring component 370 as positioned in a receptacle disposed in a bore such that the fluid enters channels via perforations of the isolated zone and generates fractures (e.g., new fractures, reactivated fractures, etc.).

In the example method 100 shown in Figs. 1 and 2, one or more grips made at least in part of degradable material may be employed. For example, consider one or more of the plug 350, the plug component 360 and the ring component 370 as including a grip or grips made at least in part of degradable material. In such an example, the ring component 370 may include a grip or grips that can accept force and/or apply force with respect to one or more other components. As an example, the plug component 360 may be made of a plurality of parts where one or more interfaces between two or more of the parts may include a grip or grips.

As an example, a degradable elastomeric material may be included in one or more downhole tools that, for example, may degrade in a manner that allows for disruption of a seal such that fluid can penetrate a component, adjoining parts, etc. Where such a component, adjoining parts, etc., are degradable, intrusion of fluid (e.g., well fluid, hydraulic fracturing fluid, water, etc.) may causes degradation thereof.

Fig. 4 shows an example of a method 400 that includes a provision block 410 for providing one or more particulate materials, a provision block 420 for providing one or more hard materials, a process block 430 for processing materials to form one or more components and a deployment block 440 for deploying one or more components, for example, as formed per the process block 430 and optionally one or more additional components.

As shown in Fig. 4, the provision block 410 can include providing one or more different types of particulate materials where at least one of the particulate materials is reactive in that it can degrade (e.g., degrade in an aqueous solution). As an example, one or more of the particulate materials may be produced by and/or subjected to one or more severe plastic deformation (SPD) processes. As an example, a material may be processed via cryomilling as an SPD process.

As an example, particulate material may be substantially spherical. For example, particulate material made from gas atomization may be substantially spherical. Such particulate material may enhance "packing" of such material (e.g., as to form a matrix, etc.).

As an example, particulate material may be classified by particle size, for example, using FEPA grit sizes or other sizes (e.g., dimension, etc.). As an example, degradable particular material may be a microgrit material, for example, of an average or median grit size of about F230 or less (e.g., consider about 53 microns based on the average of D50). As an example, consider a degradable particulate material classified with a grit size of about F1000 (e.g., about 4.5 microns based on the average of D50).

As an example, a model may consider multimodal packing. For example, consider voids of larger particles packed with smaller particles, whose voids in turn may optionally be filled with even smaller particles, etc. (e.g., a form of geometrical progression). As an example, a population of particles with a progressive particle size distribution (PSD) may be separated into populations or, for example, separate populations of particles may be combined to form a progressive PSD (e.g., optionally a continuous PSD such as a power law PSD). As an example, a PSD may be Gaussian or another type of mathematical/statistical distribution.

As an example, a packing of particles may be characterized as a disordered packing. As an example, a so-called random loose packing (RLP) may have, for uniform spheres, a packing fraction in the limit of zero gravity of about 0.44 (e.g., void fraction of about 0.56); whereas, a so-called random close packing (RCP) may have, for uniform spheres, a packing fraction of about 0.64 (e.g., void fraction of about 0.36). RCP may be considered by some to be mathematically ill-defined and rather referred to as, for example, "maximally random jammed". As to RLP, it may be considered by some to be very loose random packing, for example, as achieved by spheres slowly settling.

As shown in Fig. 4, the provision block 420 can include providing one or more different types of hard materials. As an example, a hard material can be a carbon-based material such as diamond, a ceramic material, an interstitial compound material such as tungsten carbide (WC), or other material that can form a grip that possess a hardness sufficient to impart the grip with an anchoring ability with respect to another component that can be of a lesser hardness. For example, a hard material can be of a hardness that is in excess of a hardness of a low alloy steel (LAS).

As an example, a method can include providing a blend of materials where the materials include a non-degradable material that is not degradable in an aqueous environment and an aqueous degradable alloy material. For example, the provision block 410 of the method 400 can provide the aqueous degradable alloy material and the provision block 420 can provide the non-degradable material that is not degradable in an aqueous environment, which, per the provision block 420, can be a hard material. For example, it may be a hard material that has a hardness that is in excess of a hardness of low alloy steel (LAS).

As an example, a blend of materials can include an amount of aqueous degradable alloy that is sufficient to form a matrix for an amount of non-degradable material that is not degradable in an aqueous environment. As an example, an amount of aqueous degradable alloy may be from about 10 percent by weight to about 90 percent by weight and an amount of non-degradable material that is not degradable in an aqueous environment may correspondingly be from about 90 percent by weight to about 10 percent by weight. As an example, an amount of aqueous degradable alloy may be from about 1 percent by weight to about 99 percent by weight and an amount of non-degradable material that is not degradable in an aqueous environment may correspondingly be from about 99 percent by weight to about 1 percent by weight.

As mentioned, tungsten carbide (WC) may be utilized as a hard material that may be defined as being an interstitial compound material. In particular, tungsten carbide may be referred to as being an interstitial carbide (e.g., a metal carbide where the metal is a transition metal).

An interstitial carbide can be derived from a transition metal that acts as a host lattice for the smaller carbon atoms, which occupy the interstices of the close-packed metal atoms. Interstitial carbides can be characterized by relatively high hardness and relatively high melting points (e.g., about 3,000 degrees C to about 4,000 degrees C). An interstitial carbide may be an interstitial monocarbide or a transition metal may form interstitial carbides of several stoichiometries. For example, manganese (Mn) is known to form at least five different interstitial carbides. In contrast to the ionic carbides, various interstitial carbides do not react with water and tend to be chemically inert. Tungsten carbide (WC) and tantalum carbide (TaC), possess considerable hardness and chemical inertness.

As an example, tungsten carbide (WC) may be wetted by molten nickel and may be wetted by molten cobalt. As an example, a W-C-Co system may include a pseudo binary eutectic. Tungsten carbide particles may aggregate where metallic cobalt may serve as a matrix. As an example, tungsten carbide particles can be embedded in metallic cobalt binder forming a composite. As an example, a tungsten carbide material that includes cobalt (Co) may be referred to as a cemented carbide, depending on composition.

**Table 1**

| Cemented carbide | Hardness HV (RT) | Modulus GPa | Traverse rupture strength MPa | Coefficient of thermal expansion, 10⁻⁶/K | Thermal conductivity, W/m.K | Density g/cm³ |
|---|---|---|---|---|---|---|
| WC-20 wt% Co | 1050 | 490 | 2850 | 6.4 | 100 | 13.55 |
| WC-10 wt% Co | 1625 | 580 | 2280 | 5.5 | 110 | 14.50 |
| WC-3 wt% Co | 1900 | 673 | 1600 | 5.0 | 110 | 15.25 |
| WC-10 wt% Co-22 wt% (Ti,Ta,Nb)C | 1500 | 510 | 2000 | 6.1 | 40 | 11.40 |

Tungsten carbide as WC, with a hexagonal crystal structure, can possess a hardness of about 2200 HV (50 kg) and a melting temperature of about 2800 degrees C with a density of about 15.6; while tungsten carbide as W₂C, with a hexagonal crystal structure, can possess a hardness of about 3000 HV (50 kg) and a melting temperature of about 2777 degrees C with a density of about 17.3.

As an example, a metal matrix composite (MMC) material can include from about 1 percent to about 15 percent by weight of ceramic powder(s) mixed with an aqueous degradable alloy where such a MMC material can exhibit improved hardness and higher modulus (e.g., consider an example at about 14 percent by weight). As an example, a method can include formulating a blend such that a volume percent of particulates may be greater than about 80 percent, for example, of ceramics and/or iron (Fe) based alloy powders that are bound by an aqueous degradable alloy. Such a material can be a solid with hardness adequate to bite or anchor into an LAS casing.

As an example, a non-degradable material that is not degradable in an aqueous environment can be a material that includes covalent bonds. As an example, such a material can be a network solid or covalent network solid that is a chemical compound (e.g., or element) in which atoms are bonded by covalent bonds in a continuous network extending throughout the material. For example, in a network solid there may be no substantial presence of individual molecules such that an entire crystal may be considered a macromolecule.

As an example, a network solid material can be or include diamond with a continuous network of carbon atoms and/or silicon dioxide (e.g., quartz) with a continuous three-dimensional network of SiO₂ units; noting that graphite and the mica group of silicate minerals structurally include continuous two-dimensional sheets covalently bonded within the layer, with other bond types holding the layers together.

As an example, a network solid material can be very hard due to strong covalent bonds throughout a lattice; can have a high melting point as melting means breaking covalent bonds; may be poor electrical conductors where electrons are used for sigma bonds (e.g. diamond and quartz) due to little to no delocalized electrons; can be generally insoluble (e.g. due to difficulty of solvating a very large molecule). A network solid material such as diamond or silicon dioxide can be considered to be non-degradable materials that are not degradable in an aqueous environment as may exist in a downhole environment or operation in a downhole environment.

As shown in Fig. 4, the process block 430 can include one or more processes that can form a component. For example, consider a pressing process, a casting process, etc. As an example, a process can include one or more types of surface treatment processes such as, for example, sintering and/or nitriding.

As an example, a method can include providing a blend of materials and pressing the blend of materials where the materials include a non-degradable material that is not degradable in an aqueous environment and an aqueous degradable alloy material; and forming a degradable grip from the pressed blend of materials.

As an example, a hard material can be, for example, a polycrystalline diamond material or a cubic boron nitride material. As an example, processing can include pressing such as utilized in making pieces of polycrystalline diamond (PCD) or pieces of polycrystalline cubic boron nitride (PCBN). For example, a mixture of materials can be subjected to pressing to form one or more blanks or to form one or more grips directly. As an example, a pressed blank or grip may be sintered and/or nitrided. As an example, a grip may be formed from a blank. As an example, a grip may be formed as an insert or another type of part that can be operatively coupled to another part.

As an example, a metal matrix composite (MMC) material can include a nickel-based super alloy material. In such an example, the MMC material may optionally be nitrided to impart surface properties. As an example, a degradable grip can include a nitrided surface. As an example, a nickel-based super alloy can include about 10 to about 20 percent by weight Cr, up to about 8 percent by weight Al and Ti, and about 5 to about 10 percent by weight Co. As an example, a nickel-based super alloy may include one or more amounts of one or more other elements (e.g., B, Zr, C, Mo, W, Ta, Hf, and Nb).

As an example, nitriding may be implemented as a heat treating process that acts to diffuse nitrogen into a surface of a metallic material, for example, to create a case-hardened surface. As an example, nitriding may include laser nitriding and/or anotherform of nitriding.

As an example, a pressing process may be a high pressure and high temperature (HPHT) pressing process. For example, consider one or more of a cubic press, a belt press, and a piston-cylinder press that may be capable of generating sufficiently high pressures and temperatures for forming a consolidated material such as, for example, a metal matrix composite (MMC) material that includes degradable material. As an example, consider a HPHT press that can achieve pressures of the order of about 6,900 MPa or more (e.g., about 1000 ksi or more) and, for example, temperatures of the order of 1,000 degrees C or more (e.g., about 1800 degrees F or more). As an example, a press may be utilized to sinter a mixture of materials, which may optionally include PCD, polycrystalline cubic boron nitride (PCBN) and/or one or more other types of hard material.

As an example, a cubic press can be a triaxial pressing system that can be suited to sintering products with multidimensional geometries. As an example, a belt press can include a reaction volume appropriate for single products or multiples of smaller products. As an example, a piston-cylinder press can include a high-pressure capsule contained within a cylindrical bore of a carbide die supported by radial hydraulic pressure, allowing for pressurization of the inside and outside of the die.

As an example, a degradable metal-based material can be utilized to form a matrix for a hard material to form a metal matrix composite material. In such an example, the metal matrix composite (MMC) material may be shaped as a grip that can be utilized to anchor one component with respect to another component.

As an example, a MMC material can include one or more types of ceramic powders mixed with a degradable alloy powder. Such a MMC material can be processed to form a consolidated material with enhanced hardness and modulus.

As an example, a method can include increasing a volume fraction of particulates where, for example, more than about 80 percent by volume of ceramic and/or iron-based alloy powder are bound by a degradable alloy. Such a consolidated material can possess adequate hardness to bite or anchor into a LAS casing. As an example, hardness of such a material (e.g., a MMC material) can be enhanced via nitriding. As an example, nitriding may slow near surface dissolution rate of such a material.

As an example, a MMC material may be formed into one or more shapes suitable for a grip (e.g., to anchor one component with respect to another component). As an example, a grip may be shaped as a button, shaped as teeth, shaped as a part with teeth, etc.

As an example, a tool may include one or more grooves, channels, passages, etc., that may be at least partially filled with one or more degradable materials (e.g., a degradable MMC material). In such an example, degradation may allow one component to move with respect to another component. Or, for example, degradation may occur after one or more operations to assure that a grip or grips dissolve and do not interfere with a subsequent operation or operations.

As shown in Fig. 4, the deployment block 440 can include disposing one or more components in a downhole environment and degrading at least a portion of one of the one or more components in the downhole environment. As an example, the deployment block 440 may also include ageing of one or more components in an environment or environments in which a component or components may be deployed. As an example, ageing can include heat treating.

As an example, a degradable material can be a water-reactive material that breaks down in aqueous fluids (e.g., dissolves and disintegrates into powder form, etc.). For example, a degradable MMC material can include water reactive material that forms a matrix for a hard material where exposure to water causes the water reactive material to generate hydrogen, which, as a gas, may migrate via pressure build-up through the MMC material and thereby cause breaking thereof.

As an example, one or more degradable components may be implemented in one or more tools, pieces of equipment, etc., for example, to achieve temporary anchoring (e.g., static and/or dynamic). As an example, an operation that performs multistage stimulation may employ one or more degradable elements, optionally as triggering components. For example, degradation of an element may trigger slippage of one or more components with respect to one or more other components.

Fig. 5 shows an example of a method 510 and an example of a method 550. The method 510 includes a provision block 514 for providing a powder mixture, a formation block 518 for forming one or more grips, a formation block 522 for forming an assembly and a deployment block 526 for deploying the assembly.

In the method 510, the powder mixture 514 can include a degradable alloy material and, for example, tungsten carbide. As an example, the powder mixture can include about 90 percent tungsten carbide powder by weight and about 10 percent of a degradable alloy powder by weight. As an example, the powder mixture can include about 50 percent or more tungsten carbide by weight. As an example, the powder mixture can include about 1 percent or more of degradable alloy by weight. As an example, tungsten carbide may be provided as a powder with an average grain size of about 0.6 microns. As an example, tungsten carbide may be provided as a powder with an average grain size of about one micron or less.

In the method 510, the one or more grips may be formed at least in part via pressing. For example, consider cold pressing. As an example, the one or more grips may be formed in part via a heating process. For example, consider heating powder (e.g., consolidated, pressed, unpressed, during pressing, etc.) to a temperature of the order of hundreds of degrees C or more. For example, consider heating powder during pressing to a temperature of about 1000 degrees C or more. As an example, a method can include heating material to a temperature of about 1400 degrees C. Such heating may be considered to be heat treating that may act to "glue" particles together, for example, with or without necking, etc., which may be characteristics of sintering.

As an example, the method 510 can include forming one or more grips that include tungsten carbide. As an example, a grip can be formed at least in part by pressing where the grip includes about 90 percent by weight of tungsten carbide and where the grip possesses a Vickers hardness of about 1323 HV as a Vickers pyramid number (e.g., corresponding to about 73 HRC). The Rockwell hardness C (HRC) may be defined by a process that applies about 150 kgf with an indenter that is 120 degree diamond spheroconical. Such a process may be suitable for steels with hardness (e.g., greater than about 100 HRB).

As an example, martensite can be characterized by a hardness value of about 1000 HV and, for example, diamond can be characterized by a hardness value of about 10000 HV. As an example, a grip that includes a water degradable alloy and that includes tungsten carbide can possess a hardness that is greater than that of martensite. For example, a grip formed of a mixture of powders of about 90 percent by weight tungsten carbide and about 10 percent by weight of a water degradable alloy (e.g., including aluminum and gallium) can possess a hardness of about 1000 HV or more.

As shown in Fig. 5, the method 550 includes a provision block 554 for providing a powder mixture A, a formation block 558 for forming a base from the powder mixture A, a provision block 562 for providing a powder mixture B, a formation block 566 for forming one or more grips from the base and from the powder mixture B, a formation block 570 for forming an assembly and a deployment block 574 for deploying the assembly.

In the example of Fig. 5, the base formed by the formation block 558 can include one or more recesses that can receive a portion of the powder mixture B of the provision block 562. In such an example, the powder mixture A can include a water degradable alloy and the powder mixture B can include a carbon-based material such as, for example, diamond (e.g., polycrystalline diamond (PCD)).

As an example, a grip can include a grip portion that contacts a component to "grip" the component. In such an example, the grip portion may be made of a degradable material that includes tungsten carbide. As an example, a grip portion may be bound to a base portion where the base portion and the grip portion differ as to their composition. For example, the base portion may include a degradable alloy and tungsten carbide and the grip portion may include polycrystalline diamond (PCD). In such an example, the portions may be bound to one another such that a grip is a unitary, integral piece. For example, such a piece may function to contact (e.g., "grip") another component where such contact does not cause the grip to separate into a base portion and a grip portion. Whereas, upon exposure to water, the base portion may degrade. In such an example, the grip portion may remain intact.

As an example, a non-degradable grip portion may be dimensioned such that it may be unlikely to interfere with one or more operations. For example, a grip portion may include a maximum cross-sectional dimension of about 10 mm or less and be of an axial length of about 30 mm or less. As an example, a grip portion may include a maximum cross-sectional dimension of about 5 mm or less and be of an axial length of about 15 mm or less. As an example, a grip portion may include a maximum cross-sectional dimension of about 3 mm or less and be of an axial length of about 6 mm or less. As an example, a grip can include a base portion with dimensions of about 6 mm (e.g., height) by about 6 mm (e.g., axial length) by about 7 mm (e.g., width) with a grip portion of about 2 mm (e.g., height) by about 6 mm (e.g., axial length) by about 2 mm (e.g., width).

As an example, a method can include electrical discharge machining (EDM). As an example, a method can include spark machining, spark eroding, burning, die sinking, wire burning orwire erosion. As an example, a method can include forming a desired shape electrical discharge(s). As an example, material may be removed from a workpiece (e.g., a stock piece) by a series of rapidly recurring current discharges between electrodes, for example, separated by a dielectric material and subject to an electric voltage. As an example, an electrode can be a tool-electrode and another electrode can be a workpiece-electrode.

As an example, a method can include pressing at high pressure and high temperature for form a stock piece followed machining such as, for example, EDM cutting, which may form one or more components from the stock piece. In such an example, the stock piece may be formed at least in part from tungsten carbide powder (e.g., consider a grain size of about 0.6 micron) where the stock piece includes a dissolvable powder alloy, which can be present at a lesser weight percent than the tungsten carbide powder. As an example, a stock piece can include multiple regions where, for example, one or more regions can include a hard material such as, for example, polycrystalline diamond (PCD). As an example, such hard material may form a tip, which may be part of a ridge, a tooth, etc. As an example, a grip can include multiple regions where two or more of the regions possess different compositions.

As an example, a method can include blending by weight approximately 90 percent tungsten carbide powder and approximately 10 percent a degradable alloy powder. As an example a method can include using a die/punch system that for cold pressing a mixture of tungsten carbide powder and degradable alloy powder to form a disc with one or more recesses, openings, etc. In such an example, the mixture may include cobalt. As an example, a disc may be an annular cylindrical structure with a hole that may be substantially centered with respect to a circumference of the disc. As an example, a disc may be fit into a holder (e.g., a niobium can, etc.). As an example, an opening of a disc may be filled with a powder. For example, an opening of a disc may be filled with a polycrystalline diamond (PCD) powder, which can include, for example, cobalt. As an example, a holder may be fit with a lid (e.g., a niobium lid, etc.). As an example, a holder with contents may be pressed at a specified pressure (e.g., about 50,000 bar) and be subjected to a specified temperature (e.g., about 1400 degrees C) for a specified amount of time, which may include one or more of a pressure profile with respect to time and a temperature profile with respect to time. As an example, a method can include a cycle that includes applying pressure to a holder and contents thereof and heating the holder and contents thereof. As an example, a cycle may be of the order of tens of minutes, for example, consider a cycle with a time of about 30 minutes. As an example, pressed and heated contents of a holder may form a stock piece that can be subjected to one or more processes to form one or more grips. For example, consider EDM cutting of a stock piece, which may be followed by, for example, polishing and/or another process. As an example, a grip can include a base portion and a grip portion where at least the base portion is characterized by a Vickers hardness of about 1000 or more (e.g., of about 1300 HV or more) or, for example, a Rockwell C scale hardness of about 60 or more (e.g., of about 70 HRC or more). As an example, cobalt may be present in a grip. As an example, cobalt may be at least in part continuous across an interface between a base portion and a grip portion of a grip.

As an example, one or more parameters may be adjustable for a method of forming a stock piece and/or forming a grip. For example, consider adjustment of one or more materials as to composition and/or processing. As an example, consider adjustment of one or more materials as to particle size and/or particle shape. As an example, consider adjustment of one or more materials as to density, which may be a powder related density (e.g., a tap or tapped density). As an example, a method may include adjusting an amount and/or a type of binder. For example, a base portion may include an amount of binder and a grip portion may include an amount of binder where such binder can facilitate binding of the base portion and the grip portion to one another.

As an example, a cold pressed disc can include an opening. In such an example, a cold pressed material may be positioned at least in part in the opening. For example, consider a cold pressed disc that includes tungsten carbide and a degradable alloy and a cold pressed cylinder that includes polycrystalline diamond (e.g., consider a powder with a grain size of about 0.5 to about 1 micron, etc.). As an example, a cold pressed cylinder may optionally include degradable alloy, which may be of a composition of the degradable alloy of the cold pressed disc or, for example, a degradable alloy of a different composition. As an example, the cold pressed disc can include a binder and the cold pressed cylinder can include a binder where binder of the cold pressed disc and the binder of the cold pressed cylinder can include a common binder material. As an example, a binder can be or include cobalt.

As an example, a material may be precompacted. For example, a cylinder may be precompacted prior to being received by a recess, an opening, etc. of a piece, which may be, for example, a disc. In such an example, the disc may be formed of a precompacted material. As an example, a precompacted disc and a precompacted cylinder may be compacted to form a unitary component, which may be, for example, a stock piece from which one or more grips may be formed.

As an example, a disc can include tungsten carbide and a cylinder can include tungsten carbide where a weight percent of the tungsten carbide of the disc can be the same or different than a weight percent of the tungsten carbide of the cylinder. As an example, the disc and the cylinder can include binder where the binder may bind the cylinder and the disc to form a unitary component, which may be a stock piece from which one or more grips may be formed. As an example, a binder can be or include cobalt.

As an example, dimensions of an opening and dimensions of a cylinder may be selected to form a grip that includes a base portion and a grip portion where the grip portion includes material of the cylinder.

Fig. 6 shows an example of an illustration of a metal matrix composite (MMC) material 600 that include degradable material 610 and hard material 630, which can be hard, non-degradable material. As shown, the degradable material 610 can form a matrix for the hard material 630.

As an example, more than one type of hard material and/or more than one type of degradable material may be included in a MMC material. As an example, consider ceramic powder and metallic powder as hard materials. As an example, a hard material may be a ceramic and metallic powder such as, for example, an iron-based powder. As an example, a ceramic and metallic powder can be included at a volume percentage of about 80 percent or more in a mixture that include degradable allow powder where the degradable alloy powder acts to form a matrix for the ceramic and metallic powder. Such a water reactive metal matrix composite (MMC) material can be formulated to form a grip that possesses a hardness sufficient to grip a component that is of a lesser hardness (e.g., a low alloy steel, etc.).

As an example, a MMC material part can be case hardened via nitriding to achieve sufficient hardness. As an example, nitriding may achieve a surface hardness of a part that is sufficient to bite into an LAS casing and/or act as degradable anchoring device.

Fig. 7 shows an example of a method 700 that includes a provision block 710 for providing degradable alloy particulate material, a provision block 720 for providing non-degradable particulate material, a formation block 730 for forming a degradable grip, a formation block 740 for forming an assembly, a deployment block 750 for deploying the assembly, a performance block 760 for performing one or more operations and a dissolution block 770 for dissolving the degradable grip where, for example, dissolution occurs at least in part due to exposure of the degradable grip to an aqueous solution.

Fig. 8 shows two micrographs 810 and 830 at different scales of a metal matrix composite (MMC) material that includes approximately 14 percent by weight of SiC mixed with a degradable alloy material (e.g., up to 100 percent by weight). As an example, such a MMC material may be utilized to form a grip.

Fig. 9 shows an example of a grip 900 that includes a tip 920. As an example, the grip 900 may be received by a grip seat of a component where the grip 900 can be deployed with the component as an assembly. For example, such an assembly may be deployed in a downhole environment where the tip 920 contacts another component to position the assembly. Where the grip 900 is degradable, for example, upon exposure to water (e.g., well fluid, etc.), the grip 900 may degrade, which may free the assembly.

Fig. 10 shows an example of a grip 1000 that includes a tip 1020, a base portion 1030 and a grip portion 1040 where the tip 1020 is part of the grip portion 1040. As an example, the grip 1000 may be a unitary piece that includes different materials bonded together. For example, the base portion 1030 may be of a first composition and the grip portion 1040 may be of a second composition where the first and second compositions differ. As an example, one may include a water degradable alloy while the other may be non-degradable in water. For example, the grip portion 1040 may be made of a material that is non-degradable in water yet bondable to the base portion 1030, which may be made of a material that is degradable in water. As an example, the base portion 1030 can include a degradable allow and, for example, tungsten carbide, and the grip portion 1040 can include polycrystalline diamond (PCD). As an example, a grip can be a multiple portion grip.

In the example of Fig. 10, the grip 1000 can include an interface between the base portion 1030 and the grip portion 1040 where material of the base portion 1030 and material of the grip portion 1040 are bonded. As an example, such bonding may occur responsive to, for example, pressure and/or temperature (e.g., applying pressure to and/or heating the grip 1000).

Fig. 11 shows an example of a grip 1100 that includes a tip 1120, a base portion 1130 and a grip portion 1140 where the tip 1120 is part of the grip portion 1140. Fig. 11 also shows an example of an image where an interface is visible between material of the base portion 1130 and material of the grip portion 1140.

Fig. 12 shows an example of an arrangement of components 1200, which can be an arrangement of grips 1205 where each of the grips 1205 can include a tip 1220, a base portion 1230 and a grip portion 1240 where the tip 1220 is part of the grip portion 1240.

Fig. 13 shows an example of an assembly 1300 that includes grips 1310. In such an example, at least a portion of each of the grips 1310 can include water degradable material such as, for example, a water degradable alloy. As an example, the grips 1310 can include one or more grips that include tungsten carbide. As an example, the grips 1310 can include one or more grips that include polycrystalline diamond (PCA). As an example, the grips 1310 can include one or more grips that include tungsten carbide and polycrystalline diamond. In such an example, the tungsten carbide may be present with a water degradable alloy and, for example, cobalt may be present.

As an example, polycrystalline diamond (PCD) may include a metal such as, for example, cobalt. As an example, cobalt can be a binder for polycrystalline diamond (PCD) particles.

As an example, a material can include polycrystalline diamond (PCD) and cobalt. As an example, a grip can include such a material, for example, as a grip portion, which may include a tip or tips. In such an example, a base portion of the grip can include a material that includes a degradable alloy and cobalt. In such an example, the cobalt may bond the material of the grip portion and the material of the base portion. For example, when subjected to sufficient temperature the cobalt of the grip portion and the cobalt of the base portion may become continuous across an interface between the grip portion and the base portion. As an example, a material that includes polycrystalline (PCD) and cobalt may be fused to a material that includes a degradable alloy and cobalt. In such an example, the material that includes a degradable alloy and cobalt may include tungsten carbide. For example, consider a material that includes about 90 percent by weight tungsten carbide and about 10 percent by weight of a degradable alloy (e.g., or degradable alloys) as well as an amount of cobalt. Such a material may be bonded to a material that includes polycrystalline diamond (PCD) and cobalt, for example, via a method that includes applying pressure and heat energy. As an example, heat energy may be provided to elevate the temperature of such materials to about 1000 degrees C or more. As an example, such a heat treatment may be utilized to "glue" compacted particles. As an example, a heat treatment may include sintering.

Fig. 14 shows an example of an assembly 1400 that include sets of grips 1410-1 and 1410-2. In the example of Fig. 14, the grips 1410-1 and the grips 1410-2 can include degradable grips, which may optionally include one or more non-degradable portions (e.g., consider non-degradable tip(s)). As an example, a grip can be a multiple portion grip.

Fig. 15 shows an example of an assembly 1500 that includes grips 1510. In the example of Fig. 15, the grips 1510 may be arranged about a circumference of a portion of the assembly 1500. In the example of Fig. 15, the grips 1510 can include degradable grips, which may optionally include one or more non-degradable portions (e.g., consider non-degradable tip(s)).

Fig. 16 shows an example of a disc 1600 that is made of two materials with different compositions such that grips may be made from the disc 1600 where the grips include the two materials with different compositions. For example, the disc 1600 can include an annular portion 1602 and a cylindrical portion 1604 where the annular portion 1602 is made of a first material with a first composition and the cylindrical portion 1604 is made of a second material with a second composition. In such an example, the first and second materials may include a fusible metal such as, for example, cobalt. Such a fusible metal can bond the first and second materials about an interface defined by an outer surface of the cylindrical portion 1604 and an inner surface of the annular portion 1602.

Fig. 17 shows an example of a press 1700 that can include or be operatively coupled to a controller. As an example, the press 1700 may be in an environmentally controlled chamber. For example, such a chamber may be controlled as to one or more of gas composition, humidity, temperature, pressure, etc.

In the example of Fig. 17, the press 1700 is shown as being able to press a plurality of discs such as the disc 1600 of Fig. 16. For example, the seven discs may be processed to form thirty-five grips.

While the disc 1600 of Fig. 16 shows two portions, a disc or other shaped object may be formed with two or more portions. In such an example, the two or more portions may correspond to two or more materials.

As an example, a stock piece may be machined or otherwise processed to form a grip where the stock piece includes at least two materials in at least two regions of the stock piece.

Fig. 18 shows an example of a method 1850 that includes a provision block 1854 for providing a dissolvable material (e.g., a degradable material that can degrade in an aqueous environment), a formation block 1858 for forming a base (see, e.g., the base 1859), a provision block 1862 for providing a hard material, a formation block 1866 for forming a stock composite piece (see, e.g., the stock composite piece 1867), and a formation block 1870 for forming one or more grips (see, e.g., the grips 1871) from the stock composite piece.

Fig. 19 shows various examples of grips, which may be, at least in part, degradable. As an example, consider an assembly 1910 where a component 1911 includes a grip 1912 that can anchor the component 1911 to a component 1913 (e.g., a tubular, etc.). As an example, consider an assembly 1930 where a component 1936 includes a grip 1937 that can anchor the component 1936 to a component 1938 (e.g., a tubular, etc.). As an example, consider an assembly 1950 where a component 1951 includes grips 1952 and 1957 that can anchor the component 1951 to a component 1953 (e.g., a tubular, etc.) and/or to a component 1958 (e.g., a tubular, etc.). In such an example, the grips 1952 and 1957 may differ in composition and/or processing. As an example, the grips 1952 and 1957 may be of the same composition and/or processing (e.g., method of manufacture, etc.).

In the example assemblies 1910, 1930 and 1950, a cylindrical coordinate system (r, z, □) may be utilized to describe one or more features. For example, radii may be used to define a tubular and/or a grip and, for example, an azimuthal angle or angles or arc span may be utilized to define a tubular and/or a grip.

As shown in Fig. 19, an example assembly 1960 can include a base portion 1961 with a recess 1963 that can receive at least in part a portion of a grip 1965. For example, the base portion 1961 may be akin to one of the components 1911, 1936 or 1951 and, for example, the grip 1965 may be akin to one of the grips 1912, 1937, 1952 or 1957. As an example, a grip may be a two-sided grip, for example, with a side that is an outer side to grip one component and a side that is an inner side to grip another component.

Fig. 19 also shows an example of an assembly 1970 that includes a component 1972, a component 1974 and a grip 1975. In such an example, the components 1972 and 1974 may be cylindrical or may be planar or may be of another type of geometry. As an example, a grip may be utilized with respect to cylindrical, planar or one or more other types of geometries.

In the example of Fig. 19, the grip 1975 may be fixed to the component 1972, optionally seated in a recess or recesses. As an example, the grip 1975 may include pegs and/or recesses that can operatively couple the grip 1975 to the component 1972. For example, the component 1972 may include openings that can receive pegs that extend outwardly from the grip 1975 and/or the component 1972 can include pegs that extend outwardly therefrom that can be received by openings of the grip 1975.

As an example, a slot arrangement may be utilized such that a grip may be capable of translating a desired amount. As an example, such an approach may include translating a grip to a position that may lock the grip and/or actuate one or more other mechanisms (e.g., via a sliding into place of a grip).

As an example, a grip can include a wedge shape. For example, a grip may be described in cross-section as including a sloped portion that defines at least a portion of a wedge. As an example, a narrow end of a wedge may facilitate positioning while a thick end of a wedge provide for limiting motion via gripping (e.g., traction or friction against one or more components).

As an example, a grip can include a cam shape and may optionally be rotatable. For example, a grip can be a heart-shaped cam grip or another type of shaped cam grip, which may optionally include teeth.

As an example, a grip or grips may be fit to a biasing mechanism. For example, a spring can include grips where the spring may force the grips against one or more other components. As an example, a spring may be a stabilizer spring that may be akin to a leaf spring that may extend from a tubular component to stabilize its position within another tubular component. As an example, where grips degrade (e.g., at least in part), stabilizer springs may guide a component with an ability to move the component with less friction than when the grips are present (e.g., in a non-degraded state).

As an example, a centralizer may include one or more grips. As an example, a stabilizer may include one or more grips. As an example, a downhole tool can include one or more grips. As an example, a downhole tool string can include one or more grips. As an example, a slip can include one or more grips. As an example, a grip or grips can be a gripping toothed device or assembly that can grip one or more components and, for example, locate at least one component with respect to at least one other component, for example, to axially locate at least one of the components in a borehole, etc.

As an example, a grip may degrade in stages. For example, consider teeth that degrade before a base portion of a degradable grip that supports the teeth (e.g., as a degradable grip assembly). As an example, a grip can include teeth that degrade more slowly than a base portion. As an example, a grip can include teeth that do not degrade.

As shown in Fig. 19, an assembly 1992 can include a toothed grip 1993, an assembly 1994 can include a grip surface 1995 that may extend outwardly from a surface of the assembly 1994, an assembly 1996 can include a plurality of grips 1997 that may be ridges, and an assembly 1998 can include a plurality of grips 1999 that may be buttons. As an example, a button may include a portion that is shaped substantially as a portion of a sphere, a portion of an ellipse, a portion of a cube, etc. As an example, a button can include a peg or stem, a hole or holes, a recess or recesses, etc. As an example, a button can include a grip side and a base side where, for example, the base side is adjacent to a component that can carry the button.

Fig. 20 shows an example of an assembly 2010 that includes base portions 2020-1 and 2020-2 that carry grips 2030-1 and 2030-2, respectively. As shown, the grips 2030-1 and 2030-2 include outwardly facing teeth 2031. As shown, the base portion 2020-1 includes recesses 2022 and 2024 that can provide for positioning of the grip 2030-1, for example, via inward facing teeth 2032 and an inward facing hook 2034.

As an example, the grips 2030-1 and 2030-2 may slide transversely to be positioned with respect to the base portions 2020-1 and 2020-2. As an example, a base portion may be larger than those shown in the example of Fig. 20.

In the example of Fig. 20, a Cartesian coordinate system (x, y, z) is shown where one or more features of the assembly 2010 may be described using directions, positions, etc. of the Cartesian coordinate system. As an example, the assembly 2010 may be described using one or more other coordinate systems (e.g., a cylindrical coordinate system, etc.). As an example, a grip may be described using a spherical coordinate system.

Fig. 21 shows an example of an assembly that includes a component 2110 and a sub-assembly 2130. As shown, the component 2110 includes a slot 2112 and the sub-assembly 2130 includes ring components 2140-1 and 2140-2 and wall components 2150 and 2170. In the example of Fig. 21, the wall component 2150 includes a grip 2160 with teeth 2162. As an example, the grip 2160 may be received at least in part by the slot 2112 of the component 2110 such that the component 2110 is anchored to the wall component 2150. In such an example, where one or more of the components degrade, the component 2110 may be freed, optionally still carrying the grip 2160 in the slot 2112. In such an example, the component 2110 may degrade and free the grip 2160 where the grip 2160 degrades by itself (e.g., at least in part).

As an example, the grip 2160 may include degradable material or degradable materials that are of a slower degradation rate in a solution than one or more other degradable components of the assembly of Fig. 21. For example, a degradable portion or degradable portions of the grip 2160 may be the last of the degradable components to degrade. Or, as an alternative, such portion or portions may be of a degradation rate that makes it or them the first to degrade or, for example, in a different position in a sequence of degradation of degradable components where it or they is or are neither first nor last to degrade.

In the example of Fig. 21, a cylindrical coordinate system (r, z, □) is shown where one or more features of the component 2110 and/or the sub-assembly 2130 may be described using directions, positions, angles, etc. of the cylindrical coordinate system. As an example, the component 2110 and/or the sub-assembly 2130 may be described using one or more other coordinate systems (e.g., a Cartesian coordinate system, a spherical coordinate system, etc.).

As an example, an environment in which one or more components are deployed may be a harsh environment, for example, an environment that may be classified as being a high-pressure and high-temperature environment (HPHT). A so-called HPHT environment may include pressures up to about 138 MPa (e.g., about 20,000 psi) and temperatures up to about 205 degrees C (e.g., about 400 degrees F and about 480 K), a so-called ultra-HPHT environment may include pressures up to about 241 MPa (e.g., about 35,000 psi) and temperatures up to about 260 degrees C (e.g., about 500 degrees F and about 530 K) and a so-called HPHT-hc environment may include pressures greater than about 241 MPa (e.g., about 35,000 psi) and temperatures greater than about 260 degrees C (e.g., about 500 degrees F and about 530 K). As an example, an environment may be classified based in one of the aforementioned classes based on pressure or temperature alone. As an example, an environment may have its pressure and/or temperature elevated, for example, through use of equipment, techniques, etc. For example, a SAGD operation may elevate temperature of an environment (e.g., by 100 degrees C or more; about 370 K or more).

As to degradable material, Fig. 22 shows an example of a system that can be utilized to form one or more degradable powders 2292 and 2294.

As an example, a particulate material such as, for example, a powder, may be characterized by one or more properties, parameters, dimensions, etc. As an example, a particulate material may be characterized by one or more particle sizes. Where a particle is spherical, the particle may be quantitatively defined by its diameter (e.g., or radius). Where a particle has an irregular shape that is not-spherical, a dimension may be defined by a diameter corresponding to the volume of the particle as equated to the volume of a sphere. As an example, a particle may be ellipsoidal and, for example, defined by a major axis length and/or a minor axis length.

As an example, a particle may include a shape other than spherical, ellipsoidal, etc. As an example, consider needle or rod shaped particles that may be characterized at least in part by an aspect ratio of a longest dimension to a shortest dimension (e.g., consider an aspect ratio of about 5 to 1 or more). As another example, consider plate or platelet shape particles, which may be characterized at least in part by planar dimensions and a thickness dimension.

As an example, particulate matter may be characterized at least in part by one or more of a particle population mean as an average size of a population of particles, a particle population median as a size where approximately 50 percent of the population is below and approximately 50 percent is above, and a particle population mode or modes, for example, a size with highest frequency.

As an example, particulate material may include particles that are substantially spherical in shape (e.g., optionally characterized by sphericity). In such an example, a particle may be characterized by a particle size that corresponds to a diameter (e.g., assuming spherical shape). As an example, a powder may include particles with corresponding particle sizes that are within a range of less than about 100 microns and greater than about 10 microns.

As an example, particles may include crystalline structures, for example, a particle may be greater than about 80 weight percent crystalline. In such an example, a particle may include an amorphous structure, for example, a particle may be less than about 20 weight percent amorphous and greater than about 80 weight percent crystalline.

Crystals tend to have relatively sharp, melting points as component atoms, molecules, or ions tend to be ordered with regularity (e.g., with respect to neighbors). An amorphous solid can exhibit particular characteristics, for example, upon cleaving or breaking, an amorphous solid tends to produce fragments with irregular surfaces and an amorphous solid tends to exhibit poorly defined patterns in X-ray imaging. An amorphous, translucent solid may be referred to as a glass.

Various types of materials may solidify into an amorphous form where, for example, a liquid phase is cooled with sufficient rapidity. Various solids may be intrinsically amorphous, for example, because atoms do not fit together with sufficient regularity to form a crystalline lattice or because impurities disrupt formation of a crystalline lattice. For example, although the chemical composition and the basic structural units of a quartz crystal and quartz glass are the same (e.g., SiO₂ and linked SiO₄ tetrahedra), arrangements of atoms in space are not. Crystalline quartz includes an ordered arrangement of silicon and oxygen atoms; whereas, in quartz glass, atoms are arranged relatively randomly. As an example, when molten SiO₂ is cooled rapidly (e.g., at a rate of about 4 K/min), it can form quartz glass; whereas, large quartz crystals (e.g., of the order of a centimeter or more) may have had cooling times of the order of years (e.g., thousands of years).

Aluminum crystallizes relatively rapidly; whereas, amorphous aluminum may form when liquid aluminum is cooled at a rate of, for example, about 4 × 10¹³ K/s. Thus, cooling rate of aluminum can determine how atoms arrange themselves (e.g., regularly or irregularly).

As an example, a particle may be polycrystalline, for example, composed of crystallites (e.g., grains) that can vary in size and orientation. As an example, grain size may be determined using a technique such as X-ray diffraction, transmission electron microscopy, etc.

A grain boundary may be defined as the interface between two grains in a polycrystalline material. Grain boundaries, defects in crystal structure, tend to decrease electrical and thermal conductivity of material. Grain boundaries may be sites for precipitation of one or more phases, which may be referred to as grain boundary material. Grain boundaries may disrupt motion of dislocations through a material. As an example, reduction of grain size may improve strength, for example, as described by the Hall-Petch relationship.

As an example, grain boundaries may meet at a so-called grain boundary triple point (GBTP). At a GBTP (e.g., a volumetric space), a phase or phases (e.g., of grain boundary material) may exist that differ from that of crystalline material in a grain.

As an example, a powder may include particles that include grain sizes of less than about 2 microns. As an example, grain sizes may be less than about 1 micron. As an example, average grain sizes may be less than about 0.5 microns (e.g., less than about 500 nm). As an example, average grain sizes may be less than about 200 nm. As an example, material that exists between grains may be of a dimension of an order of tens of nanometers to an order of hundreds of nanometers. As an example, material that exists between grains may be of a dimension that is less than an average grain size. For example, consider grains with an average grain size of the order of hundreds of nanometers and grain boundary material with an inter-grain spacing dimension of the order of tens of nanometers.

As an example, a powder particle may include grains that include one or more materials at their boundaries. For example, a grain may be bound by a select material at its boundaries. As an example, a grain boundary material may coat a grain such that the grain is substantially encapsulated by the grain boundary material. As an example, a grain boundary material may be described as "wetting" a grain, for example, a grain boundary material may be continuous and wet an entire surface (e.g., boundary) of a grain. As an example, a particle can include grains that are in a continuum of a grain boundary material. In such an example, the grains may be spaced from each other by the grain boundary material. As an example, a size of the boundary (or the spacing between grains) may be of the order of tens of nanometers to hundreds of nanometers. The spacing between grains (e.g., the size of the grain boundary) may be determined at least in part based on the surface tension of the grain boundary material and the grain. Thus, for example, spacing may vary depending on the material in the grain boundary and the material of the grain. As an example, strength of a powder particle may be approximated at least in part by a relationship such as, for example: ∝ $1 / \sqrt{ } \overline{d} ,$ where *d̅* is the average grain size and σ is the energy of the grain boundary.

As an example, to form a continuous grain boundary, a boundary forming component of a melt may be greater than about two percent by weight. For example, consider a melt of an aluminum alloy and gallium where the gallium is present at a weight percent greater than about two percent and less than about 20 percent (e.g., optionally less than about 10 percent, and in some examples less than about five percent). In such an example, atomization of the melt can form particles with grains that reside in a continuum of grain boundary material that includes gallium (e.g., a substantially continuous boundary material that includes gallium). In such an example, more than about 90 percent of the gallium can be preferentially segregated to the grain boundary (e.g., located within the grain boundary material). While higher percentages of gallium may optionally be included in a melt, in general, a higher the percentage of gallium can result in formation of globular nodules within a particle. Such globular nodules can result in a reduction of mechanical strength of a particle. Where a powder is to be used to form a part or a tool (e.g., a downhole tool) that is to withstand certain mechanical force(s), yet be degradable, the powder may be formed of a melt that is tailored to meet mechanical force and degradability criteria. As an example, a degradability criterion may be met by including at least about two percent by weight of a select material (e.g., or materials) in a melt. In such an example, a powder formed by the melt can be at least about two percent by weight of the select material (e.g., considering material conservation). As an example, a powder may be of at least about two percent by weight of a select material (e.g., or select materials).

As an example, a melt may include greater than about 80 percent by weight of an aluminum alloy and greater than about two percent by weight of a select material or materials. In such an example, consider as the select material, or materials, one or more of gallium, indium, tin, bismuth, and lead. As an example, a select material or materials may include one or more basic metals where, for example, basic metals include gallium, indium, tin, thallium, lead and bismuth (e.g., basic metals of atomic number of 31 or greater). As an example, grain boundary material may include aluminum, which is a basic metal with an atomic number of 13, in addition to one or more other basic metals. As an example, a basic metal may be a post-transition metal (e.g., metallic elements in the periodic table located between the transition metals (to their left) and the metalloids (to their right) and including gallium, indium and thallium; tin and lead; and bismuth). As an example, a melt may optionally include mercury, which is a transition metal (e.g., a group 12 transition metal). As an example, a powder formed of such a melt can include mercury, which may be a boundary material that bounds grains of particles of the powder. As an example, a melt may optionally include zinc, which is a transition metal (e.g., a group 12 transition metal).

As an example, a melt and a powder formed from the melt can include one or more alkali metals. For example, consider one or more of lithium, sodium, and potassium. As an example, a melt and a powder formed from the melt can include one or more alkaline earth metals. For example, consider one or more of beryllium, magnesium, calcium, strontium and barium. As an example, a powder and/or a melt may include one or more rare earth elements. As an example, a powder and/or a melt may include scandium, thallium, etc.

As an example, one or more of an alkali metal, an alkaline earth metal, or a basic metal may be used as the select material or materials for a melt. As an example, a melt may include gallium and indium. The gallium and indium may preferentially segregate to the grain boundary, for example, during a severe plastic deformation process, resulting in a desired powder particle. Materials of an aluminum alloy, such as, for example, aluminum, magnesium, silicon, copper, for example, may also appear in the grain boundary.

As an example, consider cooling a melt that includes aluminum, magnesium and gallium such that grains form with a first amount of gallium and such that at the boundaries of the grains material forms with a second amount of gallium that exceeds the first amount of gallium. In such an example, the material at the boundaries may be characterized as gallium enriched. In such an example, the amount of gallium in the grains may be negligible (e.g., grains may be formed of an aluminum alloy substantially devoid of gallium).

As an example, a material may include aluminum (e.g., melting point of about 1220 degrees F, about 660 degrees C or about 930 K), magnesium (e.g., melting point of about 1200 degrees F, about 650 degrees C or about 920 K) and gallium (e.g., melting point of about 86 degrees F, about 30 degrees C or about 300 K). Such a material may be provided in a molten state and cooled to form grains and boundaries where the boundaries are enriched in gallium (e.g., a low melting point material of the bulk material).

As an example, a material may include gallium, indium and tin. In such an example, gallium, indium (e.g., melting point of about 314 degrees F, about 157 degrees C or about 430 K) and tin (e.g., melting point of about 450 degrees F, about 232 degrees C or about 500 K) may alloy (e.g., forming a eutectic alloy with a melting point of about - 19 degrees C, about - 2 degrees F or about 250 K). Such a material may be provided in a molten state and cooled to form grains and boundaries where the boundaries are enriched in at least gallium (e.g., as an alloy of gallium, indium and tin as a low melting point material of the bulk material).

As an example, a material may include aluminum, magnesium and copper (e.g., melting point of about 1990 degrees F, about 1090 degrees C or about 1360 K). In such an example, the material may experience an increase in strength when subjected to solution heat treatment and quenching. As an example, an aluminum, magnesium and copper alloy may increase in strength and exhibit considerable ductility upon ageing at ambient temperature (e.g., about 25 degrees C or about 300 K).

As an example, an alloy may be characterized by a series designation. For example, consider the following series that include aluminum: 1000 series alloys that include a minimum of 99 weight percent aluminum content by weight, 2000 series alloys that include copper, 3000 series alloys that include manganese, 4000 series alloys that include silicon, 5000 series alloys that include magnesium, 6000 series alloys that include magnesium and silicon, 7000 series alloys that include zinc, and 8000 series alloys that include one or more other elements not covered by other series (e.g., consider aluminum-lithium alloys).

As an example, alloys that include aluminum may be represented by designations such as: 1xx.x series that include a minimum of 99 percent aluminum, 2xx.x series that include copper, 3xx.x series that include silicon, copper and/or magnesium, 4xx.x series that include silicon, 5xx.x series that include magnesium, 7xx.x series that include zinc, 8xx.x series that include tin and 9xx.x that include other elements.

As to 1000 series alloys, with aluminum of 99 percent or higher purity, such alloys may be characterized by considerable resistance to corrosion, high thermal and electrical conductivity, low mechanical properties and workability, while tending to be non-heat treatable.

As to 2000 series alloys, these include copper as an alloying element, which tends to impart strength, hardness and machinability; noting that such alloys tend to be heat treatable.

As to 3000 series alloys, these include manganese as an alloying element and they tend to have a combination of corrosion resistance and formability while tending to be non-heat treatable.

As to 5000 series alloys, these include magnesium as an alloying element, which may be, for example, optionally included along with manganese to impart a moderate-to high-strength, non-heat-treatable alloy. A 5000 series alloy may be weldable and relatively resistance to corrosion (e.g., even in marine applications).

As to 6000 series alloys, these include magnesium and silicon in various proportions to form magnesium silicide, which makes them heat treatable. Magnesium-silicon (or magnesium-silicide) alloys tend to possess good formability and corrosion resistance with high strength.

As to 7000 series alloys, these include zinc as an alloying element and, for example, when coupled with a smaller percentage of magnesium, such alloys may tend to be heat-treatable and of relatively high strength.

As an example, a material may be degradable and, for example, an alloy may be degradable (e.g., a degradable alloy). As an example, a material may degrade when subject to one or more conditions (e.g., over time). For example, consider one or more environmental conditions and/or "artificial" conditions that may be created via intervention, whether physical, chemical, electrical, etc. As an example, conditions can include temperature, pressures (e.g., including loads and forces), etc.

As an example, a degradable alloy may degrade at least in part due to presence of internal galvanic cells (e.g., that provide for galvanic coupling), for example, between structural heterogeneities (e.g. phases, internal defects, inclusions, etc.). As an example, a degradable material may resist passivation or, for example, formation of one or more stable protective layers.

As an example, a degradable alloy can include one or more alloying elements "trapped" in "solid solution". As an example, a material may include a metal such as aluminum, which may be impeded from passivating or building a resilient protective layer (e.g., aluminum oxide such as Al₂O₃).

As an example, a material can include one or more ceramics. For example, a material can include an inorganic, nonmetallic solid that includes metal, nonmetal or metalloid atoms, at least in part held in ionic and covalent bonds. A ceramic may be regular and/or irregular in structure, for example, atoms may be regularly oriented and crystalline, semi-crystalline and/or amorphous (e.g., ceramic glass). As an example, a ceramic may be an oxide (e.g., alumina, beryllia, ceria, zirconia, etc.). As an example, a ceramic may be a nonoxide (e.g., carbide, boride, nitride, silicide, etc.). As an example, a ceramic may include an oxide and a nonoxide.

As an example, a material can include one or more oxides. As an example, during processing of an alloy in the presence of oxygen, one or more oxides may form. For example, consider an alloy that includes aluminum where alumina (e.g., an aluminum oxide, Al₂O₃) forms. As another example, consider an alloy that includes silicon where silica (e.g., a silicon oxide, SiO₂) forms. As an example, an oxide may be a dispersed material in a particle. As an example, an oxide may be of a size of about 10 nm or less and optionally about 5 nm or less.

As an example, a material can include concentrations of one or more solute elements, for example, trapped in interstitial and in substitutional solid solutions. As an example, concentrations, which may be spatially heterogeneous, of such one or more solute elements, may be controlled through chemical composition, processing, etc. As an example, consider rapid cooling where solubility is higher than at ambient temperature or temperature of use.

As an example, a material may include one or more elements or phases that liquate (e.g., melt, etc.) once elevated beyond a certain temperature, pressure, etc., which for alloys may be predictable from phase diagrams, from thermodynamic calculations (e.g., as in the CALPHAD method), etc.

As an example, a material may "intentionally" fail via liquid-metal embrittlement, for example, as in an alloy that includes gallium and/or indium. As an example, a degradable material may include an alloy or alloys and possess phases that may be susceptible to creep (e.g., superplastic) deformation (e.g., under intended force, etc.), possess phases that are brittle (e.g., which may rupture in response to impact, etc.).

As an example, a degradable material may include a calcium alloy such as, for example, calcium-lithium (Ca--Li), calcium-magnesium (Ca--Mg), calcium-aluminum (Ca--Al), calcium-zinc (Ca--Zn), calcium-lithium-zinc (Ca--Li--Zn), etc. As an example, in a calcium-based alloy, lithium may be included in concentrations, for example, between about 0 to about 10 weight percent (e.g., to enhance reactivity, etc.). As an example, concentrations ranging from about 0 to about 10 weight percent of one or more of aluminum, zinc, magnesium and silver may enhance mechanical strength.

As an example, a material may include one or more magnesium-lithium (Mg--Li) alloys, for example, enriched with tin, bismuth and/or one or more other low-solubility alloying elements.

As an example, a material can include one or more alloys of aluminum. As an example, a material may include one or more of an aluminum-gallium (Al--Ga) alloy and an aluminum-indium (Al--In) alloy. As an example, a material may include one or more of an aluminum-gallium-indium (Al--Ga--In) and an aluminum-gallium-bismuth-tin (Al--Ga--Bi--Sn) alloy.

As an example, a material can include aluminum, gallium and indium. For example, consider a material with an alloy of about 80 weight percent aluminum, about 10 weight percent gallium and about 10 weight percent indium. Such a material may include Vickers microhardness (500 g) of about 32 (#1), 34 (#2), 34 (#3), 30 (#4), 35 (#5), 36 (#6) and 33 (average) and estimated strength of about 100 (MPa), 15 (ksi) and 1.5 (normalized).

As an example, as explain with respect to the method 400 of Fig. 4 and the metal matrix composite (MMC) of Fig. 5, a MMC material can be formed via a blend of an aqueous degradable alloy material and a non-degradable material, which can be included to increase hardness beyond the hardness of the aqueous degradable alloy material by itself.

A Vickers microhardness test procedure such as, for example, ASTM E-384, can specify a range of loads using a diamond indenter to make an indentation which is measured and converted to a hardness value. As an example, a square base pyramid shaped diamond can be used for testing in the Vickers scale where, for example, loads can be ranging from a few grams to one or several kilograms; noting that "macro" Vickers loads can range up to 30 kg or more.

As mentioned, as an example, AISI 4130 may have a Vickers hardness of about 207 (e.g., Brinell hardness of about 197) and a yield strength of about 435 MPa (e.g., about 63 ksi). As an example, 316L stainless steel can exhibit a Vickers hardness of about 140; whereas diamond can exhibit a Vickers hardness of about 10,000. As mentioned, as an example of another hard material, consider martensite with a Vickers hardness of about 1,000; noting that hard crystalline or polycrystalline materials may fracture rather than "indent" (e.g., exhibit an indentation fracture hardness).

As an example, a material can include aluminum, gallium and indium and a hard material to form a MMC material. For example, consider an aqueous degradable material with an alloy of about 80 weight percent aluminum, about 10 weight percent gallium and about 10 weight percent indium. In such an example, a hard material may be blended in to form a MMC material (see, e.g., Figs. 4, 5, etc.) where the MMC material may be of a Vickers hardness greater than about 40 and, for example, optionally greater than about 100, optionally greater than about 140, optionally greater than about 200, optionally greater than about 207, etc. As an example, a blend may be formulated to achieve a desired Vickers hardness of a degradable grip where, for example, the Vickers hardness is equal to or greater than that of a component to which the degradable grip is intended to grip into (e.g., forcibly contact, etc.).

As an example, a component may be formed of material that provides a desired degradation rate and desired mechanical properties (e.g., strength, elasticity, etc.). As an example, a degradation rate may depend upon one or more conditions (e.g., temperature, pressure, fluid environments), which may be exist in an environment and/or may be achieved in an environment (e.g., via one or more types of intervention). As an example, a material may be conditionally degradable (e.g., degradable upon exposure to one or more conditions).

As an example, a material may be a metal matrix composite (MMC) material, which is a composite material with at least two constituent parts, one being a metal, the other material may be a different metal or another material, such as a ceramic or organic compound. When at least three materials are present, it may be referred to as a hybrid composite. As an example, a MMC material may be complementary to a cermet.

As an example, a method may utilize one or more powder metallurgy (PM) techniques. As an example, one or more powder metallurgy techniques may be utilized to form particulate material. As an example, one or more powder metallurgy techniques may be utilized to form a blend of particulate materials. As an example, one or more powder metallurgy techniques may be utilized to form a component or components, for example, from a blend of particulate materials.

As an example, a material may be tailored as to one or more of its mechanical properties and/or its dissolution characteristics (e.g., degradation characteristics) via one or more processes, which can include one or more SPD processes. In such an example, the material may be refined as to its grain size and/or the defect structure of its grain boundaries. As mentioned, the Hall-Petch relation can exhibit a minimum size, which may be surpassed depending on desired properties and/or characteristics of a material. For example, such a material may still be strengthened when compared to a non-SPD processed material yet include a structure size that is less than the minimum Hall-Petch relation size, which may, for example, benefit dissolution (e.g., in a desired manner).

As an example, near-nanostructured or ultrafine-grained (UFG) materials may be defined as materials having grain sizes whose linear dimensions are in the range of, for example, about 100 nm to about 500 nm. Such materials may optionally be or include alloys and, for example, be formed at least in part via one or more severe plastic deformation (SPD) processes. For example, an atomized powder may be subjected to one or more SPD processes.

In contrast to coarse-grained counterparts, near-nanostructured or UFG materials may benefit from reduced size or dimensionality of near nanometer-sized crystallites as well as, for example, from numerous interfaces between adjacent crystallites.

As an example, a process can include rapid cooling to achieve a desired rate of cooling of material. As an example, a powder metallurgy (PM) process can refine features and improve properties of material. For example, grain size can be reduced because of the short time available for nuclei to grow during solidification. As an example, rapid cooling can increase one or more alloying limits in aluminum, for example, by enhancing supersaturation, which can enable greater precipitation-hardening with a reduction in undesirable segregation effects that may occur when IM alloys are over-alloyed. Moreover, elements that are low in solubility (e.g., practically insoluble) in a solid state may be soluble in a liquid state and may be relatively uniformly dispersed in powder particles during a process that employs rapid solidification. Non-equilibrium metastable phases or atom 'clusters' that do not exist in more slowly cooled ingots may be created by employing a rapid solidification rate; such phases can increase strength.

As an example, a process can include introduction of one or more features via powder surfaces, for example, as scale of particles becomes finer, surface-to-volume ratio of the particles increases.

As an example, one or more oxides can be introduced on a desired scale from powder surfaces by mechanical attrition, for example, to result in oxide dispersion strengthening (ODS).

As an example, a process may include introducing one or more carbides (B₄C, SiC, etc.). As an example, a process may include introducing one or more insoluble dispersoids (e.g., one or more materials that are practically insoluble in one or more defined environments).

As an example, a process can include cold-working powder particles by ball-milling. For example, a process can include cold-working powder particles in a cryogenic medium (e.g., or cryogenic media). Such a process can result in increased dislocation strengthening and, upon consolidation, a finer grain (and sub-grain) size which can be further stabilized by one or more ceramic dispersoids (e.g., as may be introduced during such a SPD process).

As an example, a method can include naturally ageing one or more components in a wellbore at one or more wellbore temperatures for one or more periods of time to thereby alter properties of the one or more components, which may be at least in part degradable.

As an example, a component may have an operational lifetime in a wellbore that is less than about 8 hours and then age in a manner at least in part thermally that causes the component to fail more readily. In such an example, where the component is degradable in the wellbore environment, ageing may assist with degradation, for example, via one or more failure mechanisms (e.g., elongation to failure, etc.).

As an example, a material may undergo Ostwald ripening where a portion of smaller entities dissolve and redeposit on larger entities. For example, consider small crystalline grains dissolving and constituents thereof redepositing onto larger crystalline grains such that the larger crystalline grains increase in size. Near a larger crystalline grain, a zone may exist, which may be due to a gradient or gradients in composition. As an example, intermetallic precipitates may form about a larger crystalline grain, which may be considered a macroscopic process (e.g., on a scale of about 50 microns).

As an example, a material may be treated to undergo Ostwald ripening and halo-ing to achieve desired properties, which can include dissolution rate, strength and/or ductility. For example, a haloed entity in the material may dissolve at a rate that differs from smaller entities in the material. As an example, a treatment may aim to achieve a population density of haloed entities to smaller entities, for example, to tailor one or more of dissolution rate, strength and ductility.

As an example, a water reactive or degradable powder can be blended with thermally stable nanocrystalline grains processed by cryomilling and further stabilized by inclusion of one or more types of dispersoids (e.g., SiC, B₄C, Al₂O₃, etc.).

As an example, a method can include using a blend of un-milled coarse powder(s) with a cryomilled-blend of water reactive or degradable powder (e.g., in a range of about 5 percent to about 95 percent) and one or more ceramic dispersoids (e.g., SiC, B₄C, Al₂O₃, etc.). In such an example, the average size of the water reactive powders or otherwise degradable powder is larger than the average size of the one or more ceramic dispersoids.

As an example, a method can include blending water reactive or degradable powder (e.g., in a range of about 5 percent to about 95 percent) with a material that includes thermally stable nanocrystalline grains processed by cryomilling. As an example, such a blend may be further mixed with one or more monomers, polymers, etc. to form a degradable polymeric material. In such an example, composition of the blend of powder or powders may provide for tailoring a degradable polymeric material (e.g., for a particular application, etc.).

As an example, a method can include using a blend of water reactive or degradable powder from an inert gas atomization (IGA) tank, a first cyclone and a second cyclone, for example, to help maximize yield from melt that is atomized and to help produce a multi-powder size distribution. In such an example, the blend (e.g., in a range of about 5 percent to about 95 percent) may be further blended, for example, with thermally stable nanocrystalline grains processed by cryomilling and further blended with one or more dispersoids (e.g., SiC, B₄C, Al₂O₃, etc.).

As mentioned, Fig. 22 shows an example of a system 2200 that can provide for making one or more powders 2292 and 2294. As an example, the system 2200 can process a melt 2220 using gas 2230 to form particles. In such an example, the particles may be composed of melt constituents and/or composed of melt constituents and optionally one or more gas constituents (e.g., consider oxygen in the gas 2220 forming an oxide such as alumina upon exposure to aluminum in the melt 2220). Particles formed via the system 2200 may be powder particles. The system 2200 may be considered to be a powder metallurgical system that can be implemented using powder metallurgy technology.

As shown in Fig. 22, the system 2200 includes a vacuum induction furnace 2210, an optional heat exchanger 2212 (HX), a chamber 2216, a cyclone chamber 2218, and a nozzle 2250. As illustrated, a rapid expansion of the gas 2230 as provided to the nozzle 2250 can break up the melt 2220, which may form a thin sheet and subsequently ligaments, ellipsoids and/or spheres (e.g., particles). In an example of an inert gas atomization process, particles formed may be substantially spheroidal. As an example, an atomization process may be a gas atomization process (e.g., including inert and/or non-inert gas), a water atomization process, a mechanical pulverization process, etc.

Particles may be collected in the chamber 2216 and in the cyclone chamber 2218, which can allow gas to exit and optionally recycle (e.g., with make-up gas, etc. to maintain a gas composition where multiple gases may be used). In such an example, the cyclone chamber 2218 may collect particles that are finer than the particles collected in the chamber 2216. Particles of either or both chambers 2216 and 2218 may be combined, separated, etc.

As an example, the system 2200 may include multiple cyclones, which may be in parallel and/or in series. For example, the system 2200 may include a cyclone in fluid communication with the cyclone 2218. As an example, particles collected (e.g., powder particles) may be of different size distributions, etc., depending on where the particles are collected (e.g., chamber 2216, cyclone 2218, other cyclone, etc.).

As to operational parameters of an atomization process, consider, for example, alloy composition, melt feed rate, melt temperature, melt viscosity, heat exchanger temperature (e.g., heat transfer rate, etc.), gas pressure and temperature, type of gas, nozzle geometry, etc. Gas atomization may produce particles that are substantially spherical in their shapes and that include grains and grain boundaries. As an example, gas atomization may produce particles that include crystalline structure and/or amorphous structure.

As an example, a melt temperature (see, e.g., T_{M}) may be a superheated temperature. As an example, a melt temperature may be greater than about 650 degrees C (e.g., greater than about 700 degree C and optionally greater than about 800 degrees C). As an example, a chamber such as the chamber 716 may be at a temperature of about 70 degrees C (e.g., a temperature of the order of hundreds of degrees C less than a melt temperature). As an example, gas may expand relatively adiabatically, which may facilitate cooling of melt and reducing thermal shock.

As an example, heat transfer may occur within a system such as the system 2200 such that particles are crystalline, amorphous or crystalline and amorphous.

As an example, a method may include cooling melt at a rate that causes at least a portion of a particle formed from the melt to be amorphous. For example, a method may include cooling via a cryogenic cooled target (e.g., consider the heat exchanger 2212 of the system 2200). As an example, a cryogenic cooled target may be positioned in front of an atomizing nozzle, for example, to achieve a cooling rate (e.g., Rc) where vitrification occurs for atomized (melt) droplets (e.g., to be at least in part a metallic glass structure, which may be a bulk metallic glass structure). As an example, a material may be characterized at least in part by a glass transition temperature (T_{g}) where below that temperature an amorphous material may be glassy (e.g., whereas above T_{g} it may be molten).

As an example, a method may include introduction of a gas at a low temperature. For example, consider introduction of helium in an atomization stream (e.g., introduction of helium as a gas, in a gas provided to a nozzle or nozzles).

As an example, a method may include increasing the superheating temperature of a melt, which may increase a driving force (e.g., a temperature differential) as to heat transfer (e.g., cooling). As an example, a method may include forming particles of a particular size or smaller such that heat transfer may occur more rapidly for the particles. For example, consider selecting a nozzle dimension (e.g., diameter, slit width, etc.) to achieve a particular particle size. As an example, a method may include analyzing dendrite arm spacing during cooling and adjusting one or more parameters of a gas atomization process such that amorphous particles may be formed.

As an example, a melt may be analyzed as to one or more properties such as, for example, a glass-transition or vitrification temperature (e.g., T_{g}). As an example, a system may be operated such that transformation takes place at the glass-transition temperature, T_{g}, below an equilibrium temperature for the solidification (e.g., a liquidus temperature, T_{L}), which may act to "freeze" an atomized melt in a non-equilibrium state (e.g., at least in part as an amorphous material). As an example, a liquidus temperature may be the maximum temperature at which crystals can co-exist with a melt in thermodynamic equilibrium. As an example, a method may consider a solidus temperature (Ts) that quantifies a point at which a material crystallizes. As an example, for a material, a gap may exist between its liquidus and solidus temperatures such that material can include solid and liquid phases simultaneously (e.g., akin to a slurry).

As an example, a method may include cooling a melt to produce an amorphous melt-span ribbon. In such an example, the ribbon may be further processed, for example, by mechanical crushing of the ribbon to form a powder.

As an example, a water reactive powder (e.g., a degradable powder) may be processed to form a component or components. In such an example, the powder may be produced by gas atomization (e.g., using one or more gases, optionally one or more inert gases), by ball milling, by crushing or other mechanical means, by sol-gel, etc.

As an example, a powder may include particles of one or more particle size distributions. For example, consider D90 less than about 44 microns (e.g., a mesh size of about 325), D90 less than about 60 microns, D90 less than about 90 microns, etc.

As an example, a material may be subjected to one or more SPD processes. As an example, a method can include employing one or more SPD processes.

As an example, where a method includes processing via ECAP, the method can include shearing of grains in consolidated or unconsolidated powder through a channeled die at low to high angles. As an example, ECAP can include passing material through a die (e.g., or dies) at various angles, which may abet refining of grains (e.g., of a water reactive powder), for example, to achieve a desired minimum grain size (e.g., after a certain number of ECAP passes). As an example, a method can include ECA pressing, for example, at one or more temperatures.

As an example, a method can include performing ECAP to abet refining of grains, for example, to achieve a minimum grain size (e.g., after a certain number of ECAP passes).

As an example, a method can include performing cryomilling to abet refining of grains, for example, to achieve a minimum grain size (e.g., after a certain duration of milling).

As an example, a method can include performing HPT to abet refining of grains, for example, to achieve a minimum grain size (e.g., after a certain number of HPT turns or revolutions).

As an example, a method can include performing cold working to abet refining of grains, for example, to achieve a minimum grain size (e.g., after a certain percentage of cold working).

As an example, a method may include controlling grain size. For example, consider alternating grain size from the point of inflection of an inverse Hall-Petch trend (e.g., varying for different alloys, consider about 50 nm) to an upper limit of ultrafine grains (e.g., about 1000 nm or 1 micron). As an example, a method can include controlling grain size by controlling one or more parameters of one or more SPD processes (e.g., cryomilling time, ECAP passes, HPT turns or revolutions, percentage of cold work, etc.).

As an example, a method can include processing water reactive powder via one or more SPD processes, for example, to tailor dissolution rate in a fluid, to tailor dissolution rates in various fluids, etc. As an example, a fluid may be a hydraulic fracturing fluid. As an example, a fluid may include a salt concentration or concentrations of salts. For example, consider a fluid that includes one or more of NaCl, KCl and MgCl₂. As an example, a fluid may be an aqueous fluid. Such an aqueous fluid may include one or more salts. As an example, a method may include varying percentages of one or more inhibited acid that may be used in one or more spearheading operations during hydraulic fracturing. As an example, a method can include tailoring dissolution rate (e.g., degradation rate) by controlling grain size. As an example, one or more SPD processes may be used for refining grains, for example, to achieve a minimum grain size (e.g., optionally altering grain size from the point of inflection of an inverse Hall-Petch trend).

As an example, dissolution rate (e.g., degradation rate) may be influenced by disruption of a continuous grain boundary network. One or more characteristics of such a network may be influenced by one or more SPD processes. As an example, dissolution rate (e.g., degradation rate) may be influenced by precipitation of an additional phase of dispersoids, for example, as may be processed during one or more other SPD processes.

As an example, a method can include precipitating second phase dispersoids. In such an example, the properties of such dispersoids may be influenced by choice of one or more cryogenic media. For example, consider use of one or more of liquid nitrogen and liquid argon. As an example, precipitation of second phase dispersoids may be influenced by choice of one or more grinding media. For example, consider use of one or more of low alloy/carbon steel balls, stainless steel balls, Ni alloy balls, ceramic balls, etc.

As an example, a gas atomization process can generate particles that may be characterized at least in part by size (e.g., consider a size distribution of about 10 microns to about 20 microns). In such an example, grains in particles may be of the order of about a micron. As an example, particles may be formed via gas atomization that include grains of the order of less than about one micron (e.g., optionally less than about half a micron).

As an example, a method may include one or more of the following processes and/or produce a material that includes one or more properties listed below (e.g., of a desired high strength degradable alloy): inert gas atomization (IGA) of a brittle cast melt with controlled flow through one or more nozzles (e.g., optionally of varying sizes) to yield powder particles of varying mesh size; particulate (approximately 80 percent to approximately 100 percent (e.g., approximately 90 percent) screened distribution) with sizes varying between about 10 microns and about 70 microns (e.g., between about 20 microns and about 60 microns).

Fig. 23 shows a scanning electron micrograph 2300 of particles produced via gas atomization of a brittle cast melt. Such particles may be formed by cooling the melt as it exits a nozzle (see, e.g., the nozzle 2250 of the system 2200 of Fig. 22). Such cooling may be adiabatic cooling. For example, adiabatic cooling can occur when pressure on an adiabatically isolated system is decreased, allowing it to expand, thus causing it to do work on its surroundings. When the pressure applied on a parcel of gas is reduced, the gas in the parcel is allowed to expand; as the volume increases, the temperature falls as internal energy decreases.

As an example, a gas atomization process may "capture" melt in a particle as a supersaturated solid solution. As an example, a particle may include properties that can reduce segregation of alloying constituents in solid solution. As an example, a gas atomization process may yield fine to ultrafine grain microstructure in particles that form a powder.

Fig. 23 also shows an example plot 2310 that illustrates an approximate relationship between dissolution rate and percent of a first material versus one or more other materials (e.g., a second material, a third material, etc.). As an example, a plot may exhibit one or more approximate relationships between amounts or percentages of materials and hardness and/or dissolution rate. As an example, a composite material may be formulated for making a degradable grip with a desired hardness and a desired dissolution rate when exposed to an aqueous environment (e.g., a downhole aqueous environment).

Fig. 24 shows an example of a transmission electron micrograph (TEM) 2400 of a particle of a powder. The TEM 2400 shows ultrafine grains with darker grain boundaries; noting focus ion beam (FIB) sample preparation. Specifically, the TEM 2400 shows that the particle includes grains with dimensions of the order of about one micron or less. The TEM 2400 shows various grains that include dimensions of about 0.5 microns.

As an example, a process can generate particles with grains where, for example, the processing provides for segregation of one or more low melting point constituents at grain boundaries. In such an example, the one or more low melting point constituents can coat grains and through such coating form a galvanic couple.

As an example, particles of a powder may include grain boundary interfaces where intermetallic precipitates can form during one or more ageing process, which may, for example, result in additional strengthening of the material (e.g., alloy, alloy and ceramic, etc.).

As an example, a process may provide for weakening of grain boundary interfaces in a component formed of a powder produced via gas atomization, which may help to promote embrittlement of the boundaries and further enhance a degradation mechanism (e.g., or degradation mechanisms). For example, consider a particle of a material that includes aluminum and gallium where gallium enrichment at grain boundary interfaces may promote embrittlement of the boundaries and where at least gallium interacts with fluid in a mannerthat causes degradation of the particle. As an example, a component formed of such particles (e.g., via processing of such particles) may degrade upon exposure to fluid and via embrittlement.

As an example, a material may include one or more oxide dispersoids, which may provide enhanced thermal stability and strengthening, for example, due to pinning of grain boundaries and dislocations.

As an example, differential cooling of a warm powder may abet diffusion of one or more low melting point constituents from a trapped supersaturated solid solution to a grain interior along a grain boundary, for example, causing liquid-metal embrittlement, which may enhance a degradation mechanism (e.g., consider a mechanism where gallium interacts with fluid in a manner that causes degradation).

Fig. 25 shows an example of a TEM 2500 that includes a triple junction between three grains (e.g., a GBTP) in a particle of a powder. The TEM 2500 shows contrast and compositional differences between the grain boundary and the grain; noting focus ion beam (FIB) sample preparation. The TEM 2500 includes two windows that correspond to samples: Sample 1 for grain material composition and Sample 2 for grain boundary material composition.

As an example, a method can include energy-dispersive X-ray (EDX) analysis of composition of a sample (e.g., Sample 1 of the TEM 2500 and Sample 2 of the TEM 2500). EDX is an analytical technique that can be applied for elemental analysis or chemical characterization of a sample. EDX involves interaction of a source of X-ray excitation (e.g., electrons) and a sample where, for example, a number and energy of X-rays emitted from the sample can be measured by an energy-dispersive spectrometer (e.g., EDS). As energy of X-rays can be characteristic of the difference in energy between two shells, and of the atomic structure of an element from which they were emitted, this allows the elemental composition of the sample to be measured.

As an example, in a particle, material at a grain boundary may be enriched in gallium when compared to material in a grain. As an example, in a particle, material at a grain boundary may be enriched in indium when compared to material in a grain. As an example, in a particle, material at a grain boundary may be enriched in gallium and indium when compared to material in a grain.

As an example, a particle may include material at a grain boundary that, upon analysis, generates gallium counts at one or more energies of less than about 2 keV and generates counts gallium counts at one or more energies greater than about 8 keV. In such an example, a ratio of counts may be about two to one. As an example, such a particle may include material at a grain boundary that, upon analysis, generates indium counts at energies from about 2 keV to about 5 keV. In such an example, such counts may be less than counts of a maximum gallium count at an energy greater than about 8 keV and less than counts of a maximum gallium count at an energy less than about 2 keV.

As an example, one or more ceramic and/or other particulates may be added to a powder (e.g., or powders) to form a metal matrix composites (MMC) material.

An alloy can include crystalline, amorphous or mixed structure (e.g. partially crystalline, partially amorphous). Features characterizing the structure can include grains, grain boundaries, phases, inclusions, etc. As an example, one or more features may be of the order of macroscopic, micron or submicron scale, for instance nanoscale. Shape, size, shape and size, etc. may be characteristics that can influence mechanical properties and, for example, reactivity.

As an example, a reactive material may include an element that tends to form positive ions when its compounds are dissolved in a liquid solution and whose oxides form hydroxides rather than acids with water. As an example, a material may disintegrate. For example, consider an alloy that loses structural integrity and becomes dysfunctional for instance due to grain-boundary embrittlement or dissolution of one of its elements. As an example, a byproduct of degradation from grain boundaries may not necessarily include an ionic compound such as a hydroxide and may include a metallic powder residue (e.g., consider severely embrittled aluminum alloys of gallium and indium).

As an example, a material may be electrically conductive and may include a metallic luster.

As an example, a material may be degradable and, for example, an alloy may be degradable (e.g., a degradable alloy). As an example, a material may degrade when subject to one or more conditions (e.g., over time). For example, consider one or more environmental conditions and/or "artificial" conditions that may be created via intervention, whether physical, chemical, electrical, etc. As an example, conditions can include temperature, pressures (e.g., including loads and forces), etc.

As an example, a component may be made from a blend of particulate materials that include at least one age-hardenable particulate material. In such an example, the blend can include one or more degradable particulate materials and one or more non-degradable particulate materials. As an example, a component may be age-hardened prior to deployment, during deployment and/or after deployment.

As an example, a blend of particulate materials can include an aluminum alloy that may be an age-hardenable aluminum alloy. In such an example, the blend can include particulate material that is degradable, for example, when exposed to an aqueous environment. As an example, a component may be formed of a blend of materials where the component is age-hardenable and degradable in an aqueous environment (e.g., a downhole environment that includes water).

As an example, a material can include cryomilled nanocrystalline grains, which may be thermally stable. For example, a cryomilled nano and/or UFG solid may be thermally stable up to about 0.8 of an alloy's melting point.

As an example, a method can include thermal treatment of a water reactive or degradable alloy, which may be mixed with one or more polymeric materials to form a component. Such a method may include making a blend of cryomilled and un-milled particulate material. In such an example, the method can include solution annealing, which may act to put coarse un-milled grains into solution and promote precipitate hardening during an ageing cycle in an annealed fraction. In such an example, cryomilled nano grains may be retained from going into solution due to their enhanced thermal stability, however, growth may occur to a multimodal nano and/or UFG size abetting ductility to the blended solid.

As an example, a thermal treatment (e.g., one or more of solution annealing, ageing, etc.) may be applied during and/or after formation of a consolidated polymeric material from a blend of un-milled gas atomized powder with cryomilled gas atomized (GA) powder. As an example, an un-milled GA powder can be a water reactive powder. As an example, an un-milled GA powder can be formed of a melt of a heat treatable aluminum alloy series (e.g., consider 6XXX and/or 7XXX series). As an example, a cryomilled GA powder can be water reactive powder (e.g., degradable in an aqueous environment). As an example, a cryomilled GA powder can be formed of a melt of a heat treatable aluminum alloy series (e.g., consider 6000, 7000 series). As an example, a blend can be stabilized by ceramic particulates (e.g., SiC, B₄C, Al₂O₃, etc.) to produce a metal matrix composite (MMC). In such an example, addition of ceramic particulates may be before cryomilling or, for example, during blending of un-milled and cryomilled GA powders.

As an example, a method can include blending GA powders that can have different, close or similar peak age properties and thermal cycles.

As an example, a method can include solution annealing of a bulk solid consolidated from blended cryomilled and un-milled powders. In such an example, solution annealing may aim to put un-milled component(s) (e.g., coarse grained) into solution (e.g., for a set time duration) while retaining structure of highly thermally stable cryomilled (e.g., nano grain) counterparts; noting that some grain growth may occur in nano-cryomilled grains, for example, transforming them to nano and/or ultra-fine duplex grains, which may abet additional ductility post thermal treatment.

As an example, a metal powder may be manufactured via one or more techniques, for example, depending on type of metal and alloy and desired properties. For example, a powder may be manufactured by reduction of oxides and other chemical techniques; atomization of metallic melts; pulverization of solids; electrolysis of water solutions or molten salts; etc.

As an example, dense particles of different chemical composition may be obtained by atomizing molten metal or alloys. For example, a metal stream can be atomized by process that may include one or more of atomizing in water, air, or an inert gas (e.g., argon or nitrogen).

As an example, a powder may be screened and, for example, subject to heat under a reducing atmosphere (e.g., consider surfaces of particles that are oxidized).

As an example, an atomization process may be employed to obtain one or more alloy powders, which may include an even distribution of alloying metals in the volume of each particle.

As an example, a PM alloy may circumvent segregation associated with ingot metallurgy (IM) product (casting etc.), where cooling from a molten state tends to be relatively slow, which may be detrimental to workability, etc.

In a PM process, an increased cooling rate may be employed compared to an IM process where, for example, the increased cooling rate may result in an extension of solid solubility limits that can lead to larger volume fractions of finer second-phase particles and/or formation of metastable phases.

As an example, a PM process may produce relatively homogeneous powder particles with substantial uniformity and with fine microstructure. Such characteristics may result enhanced mechanical properties.

As an example, an extension of phase fields and creation of additional phases can relate to supercooling, as achieved via one or more powder metallurgy techniques. As an example, microstructural refinement can occur in part due to reduced diffusion distances.

As an example, rapid cooling via a PM process can result in an increased tolerance to trapped elements (e.g., compared to material obtained via an IM process). For example, in a PM process, material may experience reduced segregation, especially as to sites such as grain boundaries.

As an example, a method can include blending powders from different alloys where, for example, an alloy may be age-hardenable or non-age-hardenable and/or degradable or non-degradable. As an example, an aluminum alloy may be selected from the 5000 series or from the 7000 series. As an example, a blend of powders can include particles with nanocrystalline grains. As an example, a blend of powder can include milled particles, for example, mechanically milled particles (e.g., consider cryomilling). As an example, a blend of powders can include one or more dispersoids.

As an example, a method can include tailoring dissolution of a component. For example, such a method may include blending powders of one or more non-degradable alloys with one or more degradable powders.

As an example, a method can include blending of water reactive or degradable powder with one or more other powders where the water reactive or degradable powder is in a range of about 5 percent to about 95 percent of the weight of a blend. In such an example, a powder may be an age-hardenable non-degradable powders (e.g., consider aluminum 6000 and 7000 series); may be a strain hardenable non-degradable powders (e.g., consider aluminum 5000 series, etc.); may be a powder that includes highly thermally stable nanocrystalline grains processed by cryomilling; may be a powder that includes highly thermally stable nanocrystalline grains processed by cryomilling that are further stabilized by dispersoids (e.g., SiC, B₄C, Al₂O₃, etc.), for example, to produce a metal matrix composite (MMC) material; etc.

As an example, a method can include blending water reactive or degradable powder with material that includes highly thermally stable nanocrystalline grains processed by cryomilling and optionally further blending dispersoids (e.g., SiC, B₄C, Al₂O₃, etc.).

Fig. 26 shows an example plot 2600 of component dimension versus time of degradation for various temperatures and an example of an assembly 2610 that includes components 2612,2614 and 2615 that may be made by consolidating particulate materials and example grips 2616 and 2618, which may optionally be included in an assembly such as, for example, the assembly 2610.

As indicated, degradation of a component may be determined by a physical characteristic of the component and an environmental condition such as, for example, temperature. For example, fluid at a temperature of about 120 degrees C may cause a component to degrade more rapidly than fluid at a temperature of about 66 degrees C. As an example, a component may be constructed to include one or more layers where at least one layer includes a degradable material, which may include a dimension (e.g., thickness, etc.) that is based at least in part on information such as the information of the plot 2600 of Fig. 26. As an example, a layer may be a nitrided layer and/or a sintered layer. For example, a degradable grip can include a sintered and/or a nitrided layer. As an example, a grip can include a non-degradable portion or portions.

As an example, the assembly 2610 may include one component that degrades at a rate that differs from another component. For example, the plug component 2612 (e.g., a ball, etc.) may degrade more rapidly than the plug seat component 2614 (e.g., a ring that can include a plug seat and that may act to locate the plug seat). As shown in Fig. 26, the assembly 2610 can include a plurality of pieces where such pieces may be formed according to desired dissolution rate, strength and/or ductility. As an example, one or more of the pieces of the assembly 2610 can be or include a grip. For example, the component 2614 can include grips as teeth, buttons, ridges, etc. As an example, the component 2615 may be a sub-assembly that includes one or more grips (e.g., as teeth, buttons, ridges, etc.).

As an example, equipment associated with one or more types of downhole operations can include one or more types of degradable grips. As mentioned, a liner may be a casing (e.g., a completion component). As mentioned, a liner may be installed via a liner hanger system. As an example, a liner hanger system may include various features such as, for example, one or more of the features of the example assembly 2750 of Fig. 27.

As shown in Fig. 27, the assembly 2750 can include a pump down plug 2760, a setting ball 2762, a handling sub with a junk bonnet and setting tool extension 2764, a rotating dog assembly (RDA) 2766, an extension(s) 2768, a mechanical running tool 2772, a hydraulic running tool 2774, a hydromechanical running tool 2776, a retrievable cementing bushing 2780, a slick joint assembly 2782 and/or a liner wiper plug 2784.

As an example, a plug may be an object that can be seated, for example, to seal an opening. As an example, the pump down plug 2760 and the setting ball 2762 may be plugs. As an example, a plug tool may be a tool that includes at least one seat to seat a plug. For example, a plug tool may include a seat that can seat a plug shaped as a ball (e.g., a spherical plug), as a cylinder (e.g., a cylindrical plug), or other shaped plug.

As an example, an assembly may include a liner top packer with a polished bore receptacle (PBR), a coupling(s), a mechanical liner hanger, a hydraulic liner hanger, a hydraulic liner hanger, a liner(s), a landing collar with a ball seat, a landing collar without a ball seat, a float collar, a liner joint or joints and/or a float shoe and/or a reamer float shoe.

As an example, a method can include a liner hanger setting procedure. Such a procedure may include positioning a liner shoe at a depth at which a hanger is to be set, dropping a setting ball from a ball dropping sub of a cementing manifold, gravitating or pumping the ball down to a ball catch landing collar, reducing the pump rate when the ball is expected to seat, increasing pressure, which pressure may act through setting ports of a hanger body and set slips on to a casing, and while holding the hanger setting pressure, setting the liner hanger by slacking off the liner weight on the hanger slips, where a loss of weight may be indicated on a weight gauge as the liner hanger sets.

In the foregoing example, it may be desirable that the ball (see, e.g., the ball 2762) has properties suited for one or more operation or operations. Properties may include mechanical properties and may include one or more other types of properties (e.g., chemical, electrical, etc.). As an example, it may be desirable that the ball degrades. For example, a ball may be manufactured with properties such that the ball degrades when exposed to one or more conditions (e.g., consider environmentally-assisted cracking). In such an example, where the ball acts to block a passage, upon degradation, the passage may become unblocked. As an example, a ball or other component (e.g., a plug, etc.) may degrade in a manner that facilitates one or more operations.

As an example, one or more components of the assembly 2750 can include a degradable grip or degradable grips that are made at least in part of a degradable material.

As an example, a component or a portion of a component may degrade in stages. For example, consider a plug that degrades from a first size to a second smaller size. In such an example, the second smaller size may allow the plug to move (e.g., from a first seat to a second seat, etc.). As an example, a plug tool may be a degradable tool. As an example, a plug tool may be degradable in part (e.g., consider a frangible degradable plug). For example, consider a plug tool with a degradable seat or degradable seats. In such an example, a plug may be seated in a degradable seat that upon degradation of the seat, the plug may pass through the seat (e.g., become unplugged with respect to that seat). As an example, a system can include a plug tool that is degradable at least in part and one or more degradable plugs (e.g., balls, cylinders, etc.). As an example, a layer of a plug, a seat, etc., may be a degradable polymeric material layer.

Fig. 28 shows an example of a life cycle 2810. In the life cycle 2810, various times are illustrated as to stages or phases. For example, one or more materials may be provided, a blend may optionally be made of multiple materials, and a blend may be pressed via one or more processes. As an example, a finished grip may be deployed, utilized and then, at least in part, degraded.

As an example, a component may be formed of material that provides a desired degradation rate and desired mechanical properties (e.g., strength, elasticity, etc.). As an example, a degradation rate may depend upon one or more conditions (e.g., temperature, pressure, fluid environments), which may be exist in an environment and/or may be achieved in an environment (e.g., via one or more types of intervention).

As an example, a degradable material may be suitable for use in an operation that may include stages. For example, consider a cementing operation, a fracturing operation, etc. As explained, a process may be associated with a completion where portions of the completion are constructed, managed, altered, etc. in one or more stages. For example, cementing may occur in stages that extend successively deeper into a drilled borehole and, for example, fracturing may occur in stages.

As an example, a method can include subjecting a material or materials to severe plastic deformation (SPD), for example, resulting in a high defect density and equiaxed ultrafine grain (UFG) sizes (e.g., with a dimension less than about 500 nm or, for example, less than about 300 nm) and/or nanocrystalline (NC) structures (e.g., with a dimension less than about 100 nm).

As an example, a grip may be used, for example, as a component or as a portion of a component in a stage or stages of a fracturing operation. As an example, such a grip may be used as a component or as a portion of a component in a tensile-loaded application, for example, consider a bridge plug, etc. As an example, a bridge plug may be a tool, for example, a bridge plug tool. Such a tool may include one or more seats, which may, for example, provide for seating of one or more plugs.

As an example, a process material may be formed as part of a cable. As an example, consider a degradable grip for a cable.

As an example, a component formed from processed material may be a bridge plug. A bridge plug may be a downhole tool (e.g., a type of plug tool) that can be located and set to isolate a lower part of a wellbore. As an example, a bridge plug may be permanent, degradable, retrievable, etc. As an example, a bridge plug may be tailored to enable a lower wellbore to be permanently sealed from production or temporarily isolated, for example, from a treatment conducted on an upper zone. As an example, a bridge plug can include one or more degradable grips.

A part, a component, etc. constructed of a processed material or processed materials may include be a fluid sampling bottle, a pressure housing, a pump shaft, a cable (e.g., wireline, a power cable, etc.), a bridge plug tool, a projectile (e.g., a drop ball, a dart, etc.), a drill stem stabilizer, etc.

As an example, a method can include making a centralizer using processed material. For example, a centralizer may exhibit enhanced wear resistance that can reduce surface damage and corrosion fatigue on a borehole assembly (e.g., BHA), for example, thereby increasing BHA lifetime. As an example, via improved abrasion wear resistance of a centralizer, reliability may be improved, for example, when drilling over extended deviated lengths.

As an example, a borehole tool may be a tool that is part of a borehole assembly (e.g., "BHA") or borehole system. As an example, a BHA may be a lower portion of the drillstring, including (e.g., from a bottom up in a vertical well) a bit, a bit sub, optionally a mud motor, stabilizers, a drill collar, a heavy-weight drillpipe, a jarring devices (e.g., jars) and crossovers for various threadforms. As BHA may provide force for a bit to break rock (e.g., weight on bit), survive a hostile mechanical environment and provide a driller with directional control of a borehole. As an example, an assembly may include one or more of a mud motor, directional drilling and measuring equipment, measurements-while-drilling tools, logging-while-drilling tools or other borehole tools.

As an example, an apparatus can include a shape and material that includes an aluminum alloy that has an average grain size less than about 1 micron or, for example, less than about 500 nanometers. In such an example, the apparatus may be a degradable apparatus. As an example, such an apparatus may be a degradable plug. In such an example, the degradable plug may include aluminum and gallium and, for example, indium.

As an example, a borehole tool may be a tool such as, for example, a tool operable in a downhole operation. For example, consider a plug as a tool, a plug tool, a centralizer, a sampling bottle, a wireline, a slickline, etc. As an example, one or more tools can include a degradable grip.

As an example, an alloy may include one or more of the following group 13 elements: aluminum, gallium and indium. As an example, an alloy may include at least one of the following group 2 elements: magnesium and calcium.

As an example, a method can include providing particulate material that includes an aluminum alloy where the aluminum alloy is at least approximately eighty percent by weight of the first particulate material and that includes one or more metals selected from a group of alkali metals, alkaline earth metals, group 12 transition metals, and basic metals having an atomic number equal to or greater than 31, where the one or more metals selected from the group total at least approximately two percent by weight of the particulate material. Such a particulate material may optionally be blended with one or more other particulate materials. For example, consider blending with a second particulate material that includes at least one aluminum alloy selected from a group of series 2000, 5000, 6000, 7000, and 9000.

As an example, a particulate material can include at least one basic metal having an atomic number equal to or greater than 31 where, for example, the at least one basic metal having an atomic number equal to or greater than 31 is at least approximately two percent by weight of the particulate material.

As an example, particulate material can include gallium (e.g., as a basic metal). In such an example, the gallium can be at least approximately two percent by weight of the particulate material. In such an example, the presence of gallium may make the particulate material a degradable material (e.g., degradable in an aqueous environment). For example, gallium may coat grains (e.g., as grain boundary material). As an example, a particulate material can include indium. As an example, a particulate material can include gallium and/or indium, which may be present, for example, at at least approximately two percent by weight of the particulate material.

As an example, a particulate material can include at least one group 12 transition metal selected from a group of zinc and mercury. As an example, a particulate material can include at least one of gallium, indium, tin, bismuth, zinc, mercury, lithium, sodium and potassium.

As an example, a method can include pressing a blend of materials where the materials include a non-degradable material that is not degradable in an aqueous environment and an aqueous degradable alloy material; and forming a grip from the pressed blend of materials. In such an example, the aqueous degradable alloy material can be present as a matrix that can degrade to allow for migration of the non-degradable material, for example, as particles. As an example, a non-degradable material may be localized as a portion of a grip. For example, consider a grip portion that includes one or more surfaces that are configured to contact a component for purposes of gripping the component (e.g., to position an assembly, etc.).

As an example, a degradable alloy material can include aluminum and one or more metals selected from alkali metals, alkaline earth metals, group 12 transition metals, and basic metals having an atomic number equal to or greater than 31.

As an example, a non-degradable material can be or include polycrystalline diamond (PCD). As an example, a non-degradable material can be or include polycrystalline cubic boron nitride (PCBN). As an example, a non-degradable material can be or include a network solid material. As an example, a non-degradable material can be or include a covalent network solid material. As an example, a non-degradable material can be or include a ceramic.

As an example, a non-degradable material can include a metal such as, for example, cobalt. As an example, a degradable material can include a metal such as, for example, cobalt. As an example, cobalt may provide for bonding of a degradable material and a non-degradable material.

As an example, a non-degradable material can be tungsten carbide, which can be considered to be insoluble in water. As an example, tungsten carbide can be included in a mixture with a degradable material, for example, to form a degradable component, which may be, for example, a degradable grip or a portion of a degradable grip.

As an example, a method can include pressing a blend of materials where the materials include a non-degradable material that is not degradable in an aqueous environment and an aqueous degradable alloy material; and forming a degradable grip from the pressed blend of materials to form a degradable grip with a Vickers hardness in excess of about 100 or, for example, with a Vickers hardness in excess of about 200.

As an example, a method can include pressing a blend of materials where the materials include a non-degradable material that is not degradable in an aqueous environment and an aqueous degradable alloy material; forming a degradable grip from the pressed blend of materials; and, for example, sintering the pressed blend of materials and/or nitriding the pressed blend of materials.

As an example, a method can include forming at least one degradable tooth, forming at least one degradable button, forming at least one degradable ridge, etc.

As an example, a method can include assembling at least a portion of a borehole tool using a degradable grip.

As an example, a degradable alloy material can include aluminum and one or more metals selected from a group of alkali metals, alkaline earth metals, group 12 transition metals, and basic metals having an atomic number equal to or greater than 31. In such an example, one or more metals selected from the group can include at least one basic metal having an atomic number equal to or greater than 31. In such an example, the at least one basic metal having an atomic number equal to or greater than 31 can be at least approximately two percent by weight of the degradable alloy material. As an example, one or more metals selected from the aforementioned group can include gallium.

As an example, a degradable grip can include a degradable matrix that is degradable in an aqueous environment; and non-degradable particles disposed at least in part within the matrix where the non-degradable particles are not degradable in the aqueous environment. In such an example, the degradable grip can include, for example, one or more of a tooth, a button, or other shaped feature.

As an example, a degradable grip may be of a maximum dimension less than approximately 5 cm. In such an example, the degradable grip can be an integrally formed piece of degradable material with non-degradable particulates therein (e.g., a MMC material). In such an example, the degradable grip may be formed by pressing.

As an example, an assembly can include a plurality of components where at least one of the components is or includes a degradable grip that includes a degradable matrix that is degradable in an aqueous environment and non-degradable particles disposed at least in part within the matrix where the non-degradable particles are not degradable in the aqueous environment. In such an example, the assembly can be a borehole tool.

As an example, an apparatus can include a degradable matrix that is degradable in an aqueous environment; and non-degradable particles disposed at least in part within the matrix where the non-degradable particles are not degradable in the aqueous environment. In such an example, the non-degradable particles can be or include tungsten carbide.

As an example, an apparatus can include a degradable matrix that is degradable in an aqueous environment; and non-degradable particles disposed at least in part within the matrix where the non-degradable particles are not degradable in the aqueous environment. In such an example, the apparatus can include cobalt and, for example, tungsten carbide.

As an example, an apparatus can include a degradable matrix that is degradable in an aqueous environment; and non-degradable particles disposed at least in part within the matrix where the non-degradable particles are not degradable in the aqueous environment. In such an example, the apparatus can be characterizes by a Vickers hardness of at least approximately 1000 or, for example, a Rockwell C scale hardness of at least approximately 60.

As an example, an apparatus can include a degradable matrix that is degradable in an aqueous environment; and non-degradable particles disposed at least in part within the matrix where the non-degradable particles are not degradable in the aqueous environment. In such an example, the apparatus can include a tip, which may be, for example, defined at least in part by a tip length. For example, the tip may form a ridge, a tooth, etc. where the tip extends over a length, which may be straight, curved, etc.

As an example, an apparatus can include a degradable matrix that is degradable in an aqueous environment; and non-degradable particles disposed at least in part within the matrix where the non-degradable particles are not degradable in the aqueous environment. In such an example, the non-degradable particles can be included at a weight of approximately 50 percent or more of the combined weight of the degradable matrix and the non-degradable particles; at a weight of approximately 70 percent or more of the combined weight of the degradable matrix and the non-degradable particles; or at a weight of approximately 90 percent or more of the combined weight of the degradable matrix and the non-degradable particles.

As an example, an apparatus can include a degradable matrix that is degradable in an aqueous environment; and non-degradable particles disposed at least in part within the matrix where the non-degradable particles are not degradable in the aqueous environment and where the degradable matrix includes gallium. In such an example, the gallium can be present at a weight of approximately 2 percent or more of the combined weight of the degradable matrix and the non-degradable particles.

As an example, an apparatus can include a degradable matrix that is degradable in an aqueous environment; and non-degradable particles disposed at least in part within the matrix where the non-degradable particles are not degradable in the aqueous environment. In such an example, the apparatus can be a unitary piece.

As an example, an apparatus can include a degradable matrix that is degradable in an aqueous environment; and non-degradable particles disposed at least in part within the matrix where the non-degradable particles are not degradable in the aqueous environment and where the non-degradable particles can be characterized, for example, by an average grain size of approximately one micron or less.

As an example, a grip of a downhole tool can include a degradable matrix that is degradable in an aqueous environment; and non-degradable particles disposed at least in part within the matrix where the non-degradable particles are not degradable in the aqueous environment.

As an example, a method can include pressing a blend of materials where the materials include a non-degradable material that is not degradable in an aqueous environment and an aqueous degradable alloy material; and forming a grip from the pressed blend of materials. In such an example, the degradable alloy material can include aluminum and one or more metals selected from a group of alkali metals, alkaline earth metals, group 12 transition metals, and basic metals having an atomic number equal to or greater than 31. As an example, a degradable alloy material can include gallium. As an example, a non-degradable material can be or include tungsten carbide.

As an example, an assembly can include a plurality of components where at least one of the components is a grip that includes a degradable matrix that is degradable in an aqueous environment and non-degradable particles disposed at least in part within the matrix where the non-degradable particles are not degradable in the aqueous environment and where the non-degradable particles can be or include tungsten carbide.

As an example, a component can include a degradable portion that is degradable in an aqueous environment; and a non-degradable portion that is not degradable in the aqueous environment. In such an example, the degradable portion can be a continuous volume and the non-degradable portion can be a continuous volume where an interface exists between the continuous volume of the degradable portion and the continuous volume of the non-degradable portion. In such an example, the continuous volume of the degradable portion can exceed the continuous volume of the non-degradable portion. As an example, such a component can be a unitary component.

As an example, a component can include a degradable portion that is degradable in an aqueous environment; and a non-degradable portion that is not degradable in the aqueous environment. In such an example, the degradable portion can include cobalt and the non-degradable portion can include cobalt where the cobalt includes cobalt that is continuous across an interface between the degradable portion and the non-degradable portion. As an example, an interface may be defined via a boundary of a degradable portion and a boundary of a non-degradable portion. In such an example, the boundaries may be defined in part via a base portion with an inset portion. For example, consider a base portion with an opening that can receive the inset portion. As an example, a base portion can be consolidated material that defines a recess or opening that can receive non-degradable material (e.g., as a powder, as consolidated material, etc.). In such an example, force may be applied to the base portion and the inset portion. As an example, heating may be applied to the base portion and the inset portion. As an example, force and/or heating may be applied to a base portion and an inset portion (e.g., or inset portions) to form a unitary component, which may be a stock piece that may be machined, etc. to form a plurality of individual unitary pieces that include at least a portion of the base portion and at least a portion of the inset portion.

As an example, a component can include a degradable portion that is degradable in an aqueous environment; and a non-degradable portion that is not degradable in the aqueous environment. In such an example, the non-degradable portion can include polycrystalline diamond. In such an example, the degradable portion can include gallium and, for example, tungsten carbide.

As an example, a component can include a degradable portion that is degradable in an aqueous environment; and a non-degradable portion that is not degradable in the aqueous environment. In such an example, the degradable may be characterized by a Vickers hardness of at least approximately 1000 or, for example, a Rockwell C scale hardness of at least approximately 60.

As an example, a component can include a degradable portion that is degradable in an aqueous environment; and a non-degradable portion that is not degradable in the aqueous environment. In such an example, the non-degradable portion can include a tip, which may be a ridge, a tooth, etc.

As an example, a component can include a degradable portion that is degradable in an aqueous environment; and a non-degradable portion that is not degradable in the aqueous environment. In such an example, the degradable portion can include a degradable matrix that is degradable in an aqueous environment and non-degradable particles disposed at least in part within the matrix where the non-degradable particles are not degradable in the aqueous environment. In such an example, the non-degradable particles can include tungsten carbide.

As an example, non-degradable particles of a degradable portion can be present at a weight of approximately 50 percent or more of a combined weight of a degradable matrix and the non-degradable particles. As an example, a degradable matrix of a degradable portion can include gallium where the gallium is present at a weight of approximately 2 percent or more of a combined weight of the degradable matrix and non-degradable particles (e.g., disposed substantially within the matrix).

As an example, a method can include pressing materials that include a degradable portion that includes material that is degradable in an aqueous environment and a non-degradable portion that includes material that is not degradable in the aqueous environment; and forming at least one grip from the pressed materials. In such an example, the material that is degradable can include aluminum and one or more metals selected from a group of alkali metals, alkaline earth metals, group 12 transition metals, and basic metals having an atomic number equal to or greater than 31. As an example, a material that is degradable can include gallium. As an example, a material that is non-degradable can be or include polycrystalline diamond.

As an example, an assembly can include a plurality of components where at least one of the components is a grip that includes a degradable portion that includes material that is degradable in an aqueous environment and a non-degradable portion that includes material that is not degradable in the aqueous environment. In such an example, the material that is degradable may be present in the degradable portion at a weight percent of about 50 percent or less, of about 25 percent or less, or of about 15 percent or less. As an example, a degradable portion can include gallium, tungsten carbide and cobalt and a non-degradable portion can include polycrystalline diamond and cobalt. In such an example, a portion of the cobalt may be substantially continuous across an interface between the degradable portion and the non-degradable portion. In such an example, the grip can be a unitary grip (e.g., where the degradable portion and the non-degradable portion are bound to each other).

As an example, one or more methods described herein may include associated computer-readable storage media (CRM) blocks. Such blocks can include instructions suitable for execution by one or more processors (or cores) to instruct a computing device or system to perform one or more actions. As an example, equipment may include a processor (e.g., a microcontroller, etc.) and memory as a storage device for storing processor-executable instructions. In such an example, execution of the instructions may, in part, cause the equipment to perform one or more actions (e.g., consider a controller to control processing such as ECAP, cryomilling, extruding, machining, forming, cementing, fracturing, etc.). As an example, a computer-readable storage medium may be non-transitory and not a carrier wave.

According to an embodiment, one or more computer-readable media may include computer-executable instructions to instruct a computing system to output information for controlling a process. For example, such instructions may provide for output to sensing process, an injection process, drilling process, an extraction process, an extrusion process, a pressing process, a nitriding process, a sintering process, a pumping process, a heating process, etc.

Fig. 29 shows components of a computing system 2900 and a networked system 2910. The system 2900 includes one or more processors 2902, memory and/or storage components 2904, one or more input and/or output devices 2906 and a bus 2908. According to an embodiment, instructions may be stored in one or more computer-readable media (e.g., memory/storage components 2904). Such instructions may be read by one or more processors (e.g., the processor(s) 2902) via a communication bus (e.g., the bus 2908), which may be wired or wireless. As an example, instructions may be stored as one or more modules. As an example, one or more processors may execute instructions to implement (wholly or in part) one or more attributes (e.g., as part of a method). A user may view output from and interact with a process via an I/O device (e.g., the device 2906). According to an embodiment, a computer-readable medium may be a storage component such as a physical memory storage device, for example, a chip, a chip on a package, a memory card, etc.

According to an embodiment, components may be distributed, such as in the network system 2910. The network system 2910 includes components 2922-1, 2922-2, 2922-3, ..., 2922-N. For example, the components 2922-1 may include the processor(s) 2902 while the component(s) 2922-3 may include memory accessible by the processor(s) 2902. Further, the component(s) 2922-2 may include an I/O device for display and optionally interaction with a method. The network may be or include the Internet, an intranet, a cellular network, a satellite network, etc.

### Conclusion

Although only a few examples have been described in detail above, those skilled in the art will readily appreciate that many modifications are possible in the examples. Accordingly, all such modifications are intended to be included within the scope of this disclosure as defined in the following claims. In the claims, means-plus-function clauses are intended to cover the structures described herein as performing the recited function and not only structural equivalents, but also equivalent structures. Thus, although a nail and a screw may not be structural equivalents in that a nail employs a cylindrical surface to secure wooden parts together, whereas a screw employs a helical surface, in the environment of fastening wooden parts, a nail and a screw may be equivalent structures. It is the express intention of the applicant not to invoke 35 U.S.C. § 112, paragraph 6 for any limitations of any of the claims herein, except for those in which the claim expressly uses the words "means for" together with an associated function.

## Claims

1. An apparatus comprising:
a degradable matrix that is degradable in an aqueous environment; and
non-degradable particles disposed at least in part within the matrix wherein the non-degradable particles are not degradable in the aqueous environment.

2. The apparatus of claim 1 wherein the non-degradable particles comprise tungsten carbide.

3. The apparatus of claim 2 comprising cobalt.

4. The apparatus of claim 1 comprising a Vickers hardness of at least approximately 1000.

5. The apparatus of claim 1 comprising a Rockwell C scale hardness of at least approximately 60.

6. The apparatus of claim 1 comprising a tip.

7. The apparatus of claim 6 wherein the tip comprises a tip length.

8. The apparatus of claim 1 wherein the non-degradable particles comprise a weight of approximately 50 percent or more of the combined weight of the degradable matrix and the non-degradable particles.

9. The apparatus of claim 1 wherein the non-degradable particles comprise a weight of approximately 70 percent or more of the combined weight of the degradable matrix and the non-degradable particles.

10. The apparatus of claim 1 wherein the non-degradable particles comprise a weight of approximately 90 percent or more of the combined weight of the degradable matrix and the non-degradable particles.

11. The apparatus of claim 1 wherein the degradable matrix comprises gallium.

12. The apparatus of claim 11 wherein the gallium comprises a weight of approximately 2 percent or more of the combined weight of the degradable matrix and the non-degradable particles.

13. The apparatus of claim 1 comprising a unitary piece.

14. The apparatus of claim 1 wherein the non-degradable particles comprise an average grain size of approximately one micron or less.

15. The apparatus of claim 1 comprising a grip of a downhole tool.

16. A method comprising:
pressing a blend of materials wherein the materials comprise a non-degradable material that is not degradable in an aqueous environment and an aqueous degradable alloy material; and
forming a grip from the pressed blend of materials.

17. The method of claim 16 wherein the degradable alloy material comprises aluminum and one or more metals selected from a group consisting of alkali metals, alkaline earth metals, group 12 transition metals, and basic metals having an atomic number equal to or greater than 31.

18. The method of claim 16 wherein the degradable alloy material comprises gallium.

19. The method of claim 16 wherein the non-degradable material comprises tungsten carbide.

20. An assembly comprising:
a plurality of components wherein at least one of the components comprises a grip that comprises a degradable matrix that is degradable in an aqueous environment and non-degradable particles disposed at least in part within the matrix wherein the non-degradable particles are not degradable in the aqueous environment and wherein the non-degradable particles comprise tungsten carbide.
